# EUROPEAN PATENT APPLICATION

(11) **EP 4 786 622 A1**
(43) Date of publication of application: **05.08.2026**
(21) Application number: 24872562.4
(22) Date of filing: 27.09.2024
(51) Int. Cl.: C22C 38/00, C21D 8/12, C21D 9/46, C22C 38/60, H01F 1/147, H01F 27/245, H01F 41/02

(54) **GRAIN-ORIENTED ELECTROMAGNETIC STEEL SHEET AND METHOD FOR PRODUCING GRAIN-ORIENTED ELECTROMAGNETIC STEEL SHEET**

(30) Priority: 27.09.2023 JP 2023166060
(71) Applicant: Nippon Steel Corporation, Tokyo 100-8071 (JP)
(72) Inventor: MATSUBARA, Ryo, Tokyo 100-8071 (JP); KAWAMURA, Yusuke, Tokyo 100-8071 (JP); HONMA, Rei, Tokyo 100-8071 (JP); SUZUMA, Toshiyuki, Tokyo 100-8071 (JP)
(74) Representative: Vossius & Partner Patentanwälte Rechtsanwälte mbB
(86) International application number: PCT/JP2024/034800
(87) International publication number: WO 2025/070781

(57) **Abstract**

A grain-oriented electrical steel sheet has a magnetic domain control treatment line on a surface thereof, |β_{All}|-|β_{Dr}| ≥ 0.1° is satisfied, |β_{All}| is an average value of absolute values of β angles over the entire surface of the grain-oriented electrical steel sheet, and |β_{Dr}| is an average value of absolute values of β angles at magnetic domain control points that are intersection points of a plurality of imaginary lines set at intervals of 2 mm in parallel along a rolling direction of the grain-oriented electrical steel sheet and the magnetic domain control treatment line. A method for manufacturing a grain-oriented electrical steel sheet includes: a step of acquiring a magnetic domain image of an original sheet of a grain-oriented electrical steel sheet; a step of determining a magnetic domain control treatment region based on a distribution of the spacing of magnetic domain walls in the magnetic domain image; and a step of applying magnetic domain control treatment to the magnetic domain control treatment region determined based on the distribution of the spacing of magnetic domain walls.

## Description

### TECHNICAL FIELD

The present disclosure relates to a grain-oriented electrical steel sheet and a method for manufacturing a grain-oriented electrical steel sheet.

The present application claims priority based on Japanese Patent Application No. 2023-166060 filed in Japan on September 27, 2023, the contents of which are incorporated herein by reference.

### BACKGROUND ART

The grain-oriented electrical steel sheet is a steel sheet containing 7 mass% or less of Si and having a secondary recrystallization structure in which secondary recrystallized grains are accumulated in a { 1101<001> orientation (Goss orientation) in which an easy axis of magnetization <001> is oriented in a rolling direction. Grain-oriented electrical steel sheets are mainly used as iron cores of power transformers. Grain-oriented electrical steel sheets are required to reduce energy loss (iron loss).

A technique of narrowing a spacing of magnetic domain walls of a grain-oriented electrical steel sheet (magnetic domain refinement technique by magnetic domain control treatment) for reducing iron loss has been known for a long time. The spacing of magnetic domain walls can be narrowed by irradiating the surface of the grain-oriented electrical steel sheet with a laser or an electron beam in a direction intersecting the rolling direction to introduce a thermal strain. The spacing of magnetic domain walls can also be narrowed by forming a groove in the direction intersecting the rolling direction on the surface of the grain-oriented electrical steel sheet. Examples of a method of forming the groove include a method of irradiating with a laser or an electron beam, a method by mechanical processing such as gear, and a method by chemical processing such as etching.

In recent years, in order to provide a grain-oriented electrical steel sheet having good iron loss characteristics, various improved techniques related to magnetic domain refinement have been proposed (see, for example, Patent Documents 1 to 3.).

### Citation List

### Patent Documents

Patent Document 1: Japanese Unexamined Patent Application, First Publication No. 2012-57219
Patent Document 2: Japanese Unexamined Patent Application, First Publication No. 2012-12664
Patent Document 3: Japanese Unexamined Patent Application, First Publication No. 2012-57218

### SUMMARY OF INVENTION

### Technical Problem

When the magnetic domain control treatment is applied to the grain-oriented electrical steel sheet, the magnetostrictive characteristic of the grain-oriented electrical steel sheet changes depending on the flux closure domain. As a result, noise characteristics of the grain-oriented electrical steel sheet deteriorate. The noise characteristic is a degree of noise generated by an electrical product (for example, a transformer, a motor, and the like) manufactured using a grain-oriented electrical steel sheet as a material. Magnetostriction is a phenomenon in which an outer shape is slightly deformed when a ferromagnetic material is magnetized. When the grain-oriented electrical steel sheet is excited by alternating current, the magnitude of the magnetostriction changes with a change in the strength of magnetization, and thus vibration occurs. The magnitude of the magnetostriction is very small on the order of 10⁻⁶, but the magnetostriction generates vibration in the iron core, and the vibration propagates to an external structure such as a tank of a transformer to become noise.

That is, the magnetic domain control treatment is effective for suppressing iron loss of the grain-oriented electrical steel sheet, but deteriorates noise characteristics of the grain-oriented electrical steel sheet. In recent years, there is an increasing demand for not only a reduction in iron loss but also a reduction in noise for grain-oriented electrical steel sheets. However, no magnetic domain refinement technique capable of achieving both noise reduction and iron loss reduction has been proposed so far.

An object of the present disclosure is to provide a grain-oriented electrical steel sheet capable of achieving both iron loss reduction and noise reduction, and a manufacturing method therefore.

### Solution to Problem

The gist of the present disclosure is as follows.

(1) A grain-oriented electrical steel sheet according to an aspect of the present disclosure is a grain-oriented electrical steel sheet having a magnetic domain control treatment line on a surface thereof, wherein |β_{All}|-β_{Dr}| ≥ 0.1° is satisfied, |β_{All}| is an average value of absolute values of β angles over an entire surface of the grain-oriented electrical steel sheet, and |β_{Dr}| is an average value of absolute values of β angles at magnetic domain control points that are intersection points of a plurality of imaginary lines set at intervals of 2 mm in parallel along a rolling direction of the grain-oriented electrical steel sheet and the magnetic domain control treatment line.
(2) Preferably, the grain-oriented electrical steel sheet according to (1) satisfies |β_{All}|-|β_{Dr}| ≥ 0.2°.
(3) Preferably, the grain-oriented electrical steel sheet according to (1) satisfies |β_{All}|-|β_{Dr}| ≥ 0.5°.
(4) Preferably, the grain-oriented electrical steel sheet according to (1) satisfies |β_{All}|-|β_{Dr}| ≥ 1.0°.
(5) Preferably, the grain-oriented electrical steel sheet according to any one of (1) to (4) satisfies |β_{All}|-|β_{Dr}| > σ_{All}/2, where σ_{All} is a standard deviation of the absolute value of the β angle over the entire surface of the grain-oriented electrical steel sheet.
(6) Preferably, the grain-oriented electrical steel sheet according to any one of (1) to (5) satisfies σ_{Dr} < σ_{All}, σ_{All} is a standard deviation of the absolute value of the β angle over the entire surface of the grain-oriented electrical steel sheet, and σ_{Dr} is a standard deviation of the absolute value of the β angle at the magnetic domain control point.
(7) Preferably, in the grain-oriented electrical steel sheet according to any one of (1) to (6), the magnetic domain control treatment line is a thermal strain.
(8) Preferably, in the grain-oriented electrical steel sheet according to any one of (1) to (7), the magnetic domain control treatment line is a groove.
(9) Preferably, in the grain-oriented electrical steel sheet according to (7), the absolute maximum value of the tensile strength introduced into the thermal strain in the magnetic domain control treatment line is non-uniform at each measurement point of the tensile strength.
(10) Preferably, in the grain-oriented electrical steel sheet according to (9), σ²(TSₘ) > 5.0 is satisfied, TSₘ is the tensile strength in a unit of MPa introduced into the thermal strain measured at each of a plurality of the magnetic domain control points, and σ²(TSₘ) is a variance of TSₘ.
(11) Preferably, in the grain-oriented electrical steel sheet according to (9) or (10), TS_{m(β < βDr)} > TS_{m(β ≥ βDr)} is satisfied, TS_{m(β < βDr)} is an arithmetical mean value of the absolute maximum value of the tensile strength in a unit of MPa introduced in the thermal strain measured at each of the magnetic domain treatment points having a β angle of less than β_{Dr} among the magnetic domain treatment points, and TS_{m(β ≥ βDr)} is an arithmetical mean value of the absolute maximum value of the tensile strength in a unit of MPa introduced into the thermal strain measured at each of the magnetic domain treatment points having the β angle of β_{Dr} or more.
(12) Preferably, in the grain-oriented electrical steel sheet according to (8), the absolute maximum value of the depth of the groove in the magnetic domain control treatment line is non-uniform at each measurement point of the groove.
(13) Preferably, the grain-oriented electrical steel sheet according to (12), σ²(Dₘ) > 3.0 is satisfied, Dₘ is an absolute maximum value of a depth of the grooves in a unit of µm at the magnetic domain control point, and σ²(Dₘ) is the variance of Dₘ.
(14) Preferably, in the grain-oriented electrical steel sheet according to (12) or (13), D_{m(β < βDr)} > D_{m(β ≥ βDr)} is satisfied, D_{m(β < βDr)} is an arithmetical mean value of absolute maximum values of the depths of the grooves in a unit of µm measured at each of the magnetic domain control points having a β angle of less than β_{Dr} among the magnetic domain control points, and D_{m(β ≥ βDr)} is an arithmetical mean value of absolute maximum values of the depths of the grooves in a unit of µm measured at each of the magnetic domain control points having the β angle of β_{Dr} or more.
(15) A method for manufacturing a grain-oriented electrical steel sheet according to another aspect of the present disclosure includes : a step of acquiring a magnetic domain image of an original sheet of a grain-oriented electrical steel sheet; a step of determining a magnetic domain control treatment region based on a distribution of the spacing of magnetic domain walls in the magnetic domain image; and a step of applying a magnetic domain control treatment to the magnetic domain control treatment region determined based on a distribution of a spacing of magnetic domain walls; in the grain-oriented electrical steel sheet to which the magnetic domain control treatment is applied, |β_{All}|-|β_{Dr}| ≥ 0.1° is set, and |β_{All}| is an average value of absolute values of β angles over an entire surface of the grain-oriented electrical steel sheet to which the magnetic domain control treatment is applied, and |β_{Dr}| is an average value of absolute values of β angles at magnetic domain control points that are the intersection points of a plurality of imaginary lines set at intervals of 2 mm in parallel along a rolling direction of the grain-oriented electrical steel sheet to which the magnetic domain control treatment is applied and a magnetic domain control treatment line formed by the magnetic domain control treatment.
(16) Preferably, in the method for manufacturing a grain-oriented electrical steel sheet according to (15), a region where the spacing of magnetic domain walls is a predetermined value or more is set as the magnetic domain control treatment region.
(17) Preferably, in the method for manufacturing a grain-oriented electrical steel sheet according to (15) or (16), the distribution of the spacing of magnetic domain wallss is derived from the magnetic domain image using two-dimensional Fourier transform.
(18) Preferably, in the method for manufacturing a grain-oriented electrical steel sheet according to (15) or (16), the magnetic domain control treatment is applied by irradiation with a laser or an electron beam.
(19) Preferably, in the method for manufacturing a grain-oriented electrical steel sheet according to (15), a magnetic domain control strength is made non-uniform in the step of applying the magnetic domain control treatment to the magnetic domain control treatment region.

### Advantageous Effects of Invention

According to the present disclosure, it is possible to provide a grain-oriented electrical steel sheet capable of achieving both iron loss reduction and noise reduction, and a method for manufacturing the same.

### BRIEF DESCRIPTION OF DRAWINGS

[FIG. 1] A plan view of a grain-oriented electrical steel sheet according to an embodiment of the present disclosure.
[FIG. 2] A plan view of a normal grain-oriented electrical steel sheet.
[FIG. 3] A graph illustrating a relationship between a β angle and a spacing of magnetic domain walls.
[FIG. 4A] A graph illustrating an example of distribution of the spacing of magnetic domain walls of a grain-oriented electrical steel sheet before a magnetic domain control treatment.
[FIG. 4B] A graph illustrating an example of distribution of the spacing of magnetic domain walls of a grain-oriented electrical steel sheet after a magnetic domain control treatment.
[FIG. 4C] A graph illustrating a difference between FIGS. 4A and 4B.
[FIG. 5] A graph illustrating a relationship between a spacing of magnetic domain walls before a magnetic domain control treatment and a spacing of magnetic domain walls after the magnetic domain control treatment.
[FIG. 6] A block diagram illustrating an example of a hardware constitution of the image acquisition device.
[FIG. 7] A block diagram illustrating an example of a hardware constitution of an analysis device.
[FIG. 8] A schematic diagram illustrating an example of a constitution of a laser irradiation device.
[FIG. 9] A flowchart illustrating a method for manufacturing a grain-oriented electrical steel sheet according to an embodiment of the present disclosure.
[FIG. 10] A schematic view showing a method of cutting out a plurality of partial regions from a magnetic domain image of a grain-oriented electrical steel sheet.
[FIG. 11] An example of a plurality of partial Fourier images obtained by applying two-dimensional Fourier transform to each of a plurality of partial regions cut out from a magnetic domain image of a grain-oriented electrical steel sheet.
[FIG. 12] A plan view of an original sheet of a grain-oriented electrical steel sheet.
[FIG. 13] An explanatory diagram of an imaginary line VL1 and an imaginary line VL2 set at the time of calculating |β_{All}|.
[FIG. 14] A plan view of a grain-oriented electrical steel sheet according to an embodiment of the present disclosure.
[FIG. 15] A graph schematically showing a relationship between the size of spacing of magnetic domain walls and the magnetic domain control saturation strength.
[FIG. 16] A graph schematically showing a relationship between the magnitude of β angle and the magnetic domain control saturation strength.
[FIG. 17] A schematic cross-sectional view of a grain-oriented electrical steel sheet in which a magnetic domain control treatment line is a thermal strain.
[FIG. 18] A schematic cross-sectional view of a grain-oriented electrical steel sheet in which magnetic domain control treatment lines are grooves.
[FIG. 19] A schematic plan view for explaining a method of measuring a magnetic domain control strength at an intersection point of a magnetic domain control treatment line and an imaginary line when the magnetic domain control treatment line is a thermal strain.
[FIG. 20] A schematic plan view for explaining a method of measuring the magnetic domain control strength at an intersection point of a magnetic domain control treatment line and an imaginary line when the magnetic domain control treatment line is a groove.

### DESCRIPTION OF EMBODIMENTS

### (1. Grain-oriented electrical steel sheet 1)

The grain-oriented electrical steel sheet 1 according to the present embodiment has a magnetic domain control treatment line 11 on the surface thereof, and satisfies |β_{All}|-|β_{Dr}| ≥ 0.1°. |β_{All}| is an average value of absolute values of β angles over the entire surface of the grain-oriented electrical steel sheet 1. |β_{Dr}| is an average value of absolute values of β angles at the magnetic domain control points VP2, which are the intersection points of a plurality of imaginary lines VL3 set at intervals of 2 mm in parallel along the rolling direction RD of the grain-oriented electrical steel sheet 1 and the magnetic domain control treatment line 11.

### (Magnetic domain control treatment line 11)

A plurality of the magnetic domain control treatment lines 11 provided on the surface of the grain-oriented electrical steel sheet 1 have a function of refining a 180° magnetic domain. By refining the magnetic domain, the iron loss of the grain-oriented electrical steel sheet 1 can be reduced. The magnetic domain is a collection of magnetic dipoles existing inside a ferromagnetic material, and is a small region where magnetic moments are aligned in one direction. The 180° magnetic domain is a magnetic domain in which the magnetization direction is the <100> orientation of the crystal and which is sandwiched between two 180° magnetic walls substantially parallel to the rolling direction RD. A distance (domain wall interval) between adjacent domain walls of the 180° magnetic domain is referred to as a spacing of the 180° magnetic domain walls. Hereinafter, unless otherwise specified, the spacing of the 180° magnetic domain walls is simply referred to as "spacing of magnetic domain walls".

Suitable examples of the magnetic domain control treatment line 11 are a thermal strain and/or a groove. By refining the magnetic domain, the iron loss of the grain-oriented electrical steel sheet 1 can be suppressed. However, the magnetic domain control treatment line 11 changes the magnetostrictive characteristic of the grain-oriented electrical steel sheet 1 according to the flux closure domain. As a result, noise characteristics of the grain-oriented electrical steel sheet 1 deteriorate.

The magnetic domain control treatment line 11 is formed in a direction intersecting the rolling direction RD of the grain-oriented electrical steel sheet 1. In the general grain-oriented electrical steel sheet 1 as exemplified in FIG. 2, the magnetic domain control treatment line 11 is formed over the entire width of the grain-oriented electrical steel sheet 1. However, in the grain-oriented electrical steel sheet 1 according to the present embodiment as exemplified in FIG. 1, it is not essential to provide the magnetic domain control treatment line 11 over the entire width of the grain-oriented electrical steel sheet 1. At least some of the magnetic domain control treatment lines 11 are interrupted in a region 12B where the β angle is large to be described later.

In the grain-oriented electrical steel sheet 1 illustrated in FIG. 1, the magnetic domain control treatment line 11 is a straight line. On the other hand, the magnetic domain control treatment line 11 may be a curve. The magnetic domain control treatment line 11 may have a shape having a straight line portion and a bent portion. The magnetic domain control treatment line 11 may be provided on one surface or both surfaces of the grain-oriented electrical steel sheet 1. When the magnetic domain control treatment line 11 is provided on both surfaces of the grain-oriented electrical steel sheet 1, various aspects of the grain-oriented electrical steel sheet 1 according to the present embodiment may be applied to at least one surface of the grain-oriented electrical steel sheet 1.

### (β angle)

In the grain-oriented electrical steel sheet 1 according to the present embodiment, the values |β_{All}| and |β_{Dr}| calculated by measuring the β angles satisfy a predetermined relational expression. The β angle is a deviation angle of crystal grains from the Goss orientation about the axis in the transverse direction TD. It is known that controlling the β angle is effective for controlling the magnetic characteristics of the grain-oriented electrical steel sheet 1. The deviation angle of the crystal grains from the Goss orientation about the axis in the rolled surface normal direction ND is referred to as an α angle, and the deviation angle of the crystal grains from the Goss orientation about the axis in the rolling direction RD is referred to as a γ angle.

As shown in FIG. 3, in the grain-oriented electrical steel sheet 1 (original sheet 2 described later) before the magnetic domain control treatment, there is a close relationship between the β angle and the spacing of magnetic domain walls. FIG. 3 is a graph illustrating an example of the relationship between the β angle of the grain-oriented electrical steel sheet 1 before the magnetic domain control treatment and the average value of the spacing of magnetic domain walls. In the grain-oriented electrical steel sheet 1 before the magnetic domain control treatment, the smaller the β angle, the wider the spacing of magnetic domain walls. However, in the grain-oriented electrical steel sheet 1 after the magnetic domain control treatment, the relationship illustrated in FIG. 3 is not established. This is because the magnetic domain control treatment decreases the spacing of magnetic domain walls in the region where the spacing of magnetic domain walls is wide before the magnetic domain control, but does not change the orientation (α angle, β angle, γ angle) of the crystal grains.

### (|β_{All}|-|β_{Dr}|)

The grain-oriented electrical steel sheet 1 according to the present embodiment satisfies |β_{All}|-|β_{Dr}| ≥ 0.1°. |β_{All}| is an average value of absolute values of β angles over the entire surface of the grain-oriented electrical steel sheet 1. |β_{Dr}| is an index of a β angle in the magnetic domain control treatment line 11. Specifically,|β_{Dr}| is an average value of absolute values of β angles at the magnetic domain control points VP2, which are the intersection points of a plurality of imaginary lines VL3 set at intervals of 2 mm in parallel along the rolling direction RD of the grain-oriented electrical steel sheet 1 and the magnetic domain control treatment line 11. |β_{Dr}| is obtained by averaging the absolute values of the β angles measured at each of a plurality of the magnetic domain control points VP2. Details of the method of measuring |β_{All}l and |β_{Dr}| will be described later.

When the grain-oriented electrical steel sheet 1 satisfies |β_{All}|-|β_{Dr}| ≥ 0.1°, the magnetic domain control treatment line 11 is preferentially provided in the region 12A where the β angle is small. Generally, the grain-oriented electrical steel sheet 1 has a region 12A where the β angle is small and a region 12B where the β angle is large. In the grain-oriented electrical steel sheet 1 schematically illustrated in FIG. 1, the magnetic domain control treatment line 11 is preferentially arranged in a region 12A where the β angle is small. Therefore, |β_{Dr}|, which is an index of the β angle in the magnetic domain control treatment line 11, is smaller than the average value |β_{All}| of the β angles over the entire surface of the grain-oriented electrical steel sheet 1. On the other hand, in the normal grain-oriented electrical steel sheet 1 shown in FIG. 2, the magnetic domain control treatment lines 11 are arranged without considering the distribution of the β angles. Therefore, |β_{Dr}|, which is an index of the β angle in the magnetic domain control treatment line 11, is substantially the same value as the average value |β_{All}| of the β angles over the entire surface of the grain-oriented electrical steel sheet 1.

### (Basic principle and operation and effects)

The present inventors have found that, according to the grain-oriented electrical steel sheet 1 satisfying |β_{All}|-|β_{Dr}| ≥ 0.1°, both iron loss and noise can be reduced. This is because, in the grain-oriented electrical steel sheet 1 satisfying |β_{All}|-|β_{Dr}| ≥ 0.1°, the magnetic domain control treatment line 11 is provided in the region 12A where the β angle is small, that is, the region having a wide spacing of magnetic domain walls before the magnetic domain control treatment, while the magnetic domain control treatment for the region 12B where the β angle is large, that is, the region having a narrow spacing of magnetic domain walls before the magnetic domain control treatment is suppressed. Hereinafter, the basic principle and operation and effects of the present disclosure will be described with reference to FIGS. 4A to 4C and the like.

First, the present inventors compared the magnetic domain structure of the grain-oriented electrical steel sheet 1 before and after the magnetic domain control treatment. FIG. 4A shows an example of distribution of the spacing of magnetic domain walls of the grain-oriented electrical steel sheet 1 before the magnetic domain control treatment. FIG. 4B illustrates the distribution of the spacing of magnetic domain walls after the magnetic domain control treatment is performed on the surface of the grain-oriented electrical steel sheet 1 of FIG. 4A. The magnetic domain control treatment here is performed by applying continuous wave laser irradiation along a direction substantially perpendicular to the rolling direction RD. The distribution of the spacing of magnetic domain walls shown in FIGS. 4A and 4B is derived from the magnetic domain image of the grain-oriented electrical steel sheet 1 using two-dimensional Fourier transform described later.

FIG. 4C illustrates a difference between FIGS. 4A and 4B. FIG. 4C illustrates a region refined to a spacing of magnetic domain walls of 50 µm or more before and after the magnetic domain control treatment illustrated in FIGS. 4A and 4B. According to FIG. 4C, the region in which the spacing of magnetic domain walls is refined by the magnetic domain control treatment is visualized.

According to FIG. 4C, it can be seen that the region where the magnetic domain refinement of 50 µm or more has occurred by the magnetic domain control treatment is the dark color part of FIG. 4A, that is, the region where the spacing of magnetic domain walls is wide before the magnetic domain control treatment. In particular, it can be seen that the magnetic domain refinement effect remarkably appears in a region where the original spacing of magnetic domain walls is about 500 µm or more. On the other hand, in the bright color portion of FIG. 4A, that is, in the region where the spacing of magnetic domain walls is narrow before the magnetic domain control treatment, the effect of the magnetic domain control treatment hardly appears. The effect of the magnetic domain control treatment varies depending on the spacing of magnetic domain walls before the magnetic domain control treatment.

The present inventors investigated in more detail the relationship between the reduction amount of the spacing of magnetic domain walls caused by the magnetic domain control treatment and the spacing of magnetic domain walls before the magnetic domain control treatment. FIG. 5 shows the relationship between the spacing of magnetic domain walls before the magnetic domain control treatment and the spacing of magnetic domain walls before the magnetic domain control treatment at the same position. The magnetic domain control treatment was performed by laser irradiation. At the time of laser irradiation, the average irradiation energy density Ua (mJ/mm²) and the irradiation pitch PL (mm) were set to Ua = 1.5 rnJ/mm² and PL = 4 mm, respectively.

According to FIG. 5, it can be seen that the magnetic domain refinement effect by the magnetic domain control treatment is less likely to appear in the region where the spacing of magnetic domain walls is narrow. In particular, in the region where the spacing of magnetic domain walls was about 500 µm or less, the spacing of magnetic domain walls were substantially the same before and after the magnetic domain control treatment. Therefore, it is considered that the effect of reducing the iron loss by the magnetic domain control treatment is large in a region where the spacing of magnetic domain walls before magnetic domain control is wide, but is not sufficiently obtained in a region where the spacing of magnetic domain walls before magnetic domain control is narrower than a predetermined value. It is considered that the magnetic domain control treatment line 11 formed in a region where the spacing of magnetic domain walls is narrower than a predetermined value causes deterioration of noise characteristics due to the flux closure domain.

According to the above findings, in the conventional magnetic domain control treatment of the grain-oriented electrical steel sheet 1, the magnetic domain control is performed to a portion where the magnetic domain control is unnecessary, and this contributes to an increase in noise. In addition, it is found that it is extremely effective to preferentially perform the magnetic domain control treatment in a region having a wide spacing of magnetic domain walls in order to achieve both iron loss reduction and noise reduction. Magnetic domain control treatment in a region having a wide spacing of magnetic domain walls can reduce iron loss. In addition, by minimizing the magnetic domain control treatment in a region where the spacing of magnetic domain walls is narrow, deterioration of noise characteristics can be prevented.

As shown in FIG. 3, there is a close relationship between the spacing of magnetic domain walls before the magnetic domain control treatment and the β angle. The region 12A where the β angle is small substantially coincides with a region having a wide spacing of magnetic domain walls before the magnetic domain control treatment. Therefore, the grain-oriented electrical steel sheet 1 in which the magnetic domain control treatment line 11 is preferentially provided in the region 12A where the β angle is small, and |β_{All}|-|β_{Dr}| ≥ 0.1° is satisfied is the grain-oriented electrical steel sheet 1 in which the magnetic domain control treatment is preferentially performed in the region having a large spacing of magnetic domain walls. In other words, in the grain-oriented electrical steel sheet 1 satisfying |β_{All}|-|β_{Dr}| ≥ 0.1°, both iron loss reduction and noise reduction can be achieved by preferentially performing magnetic domain control treatment on a region having a wide spacing of magnetic domain walls.

The most basic aspect of the grain-oriented electrical steel sheet 1 according to the present embodiment has been described above. Hereinafter, a more preferred aspect will be described.

### (Preferred numerical value range of |β_{All}|-|β_{Dr}|)

The larger |β_{All}|-|β_{Dr}| is, the more preferable it is from the viewpoint of improving noise characteristics. It is more preferable that |β_{All}|-|β_{Dr}| is, for example, 0.2° or more, 0.5° or more, or 1.0° or more. That is, it is more preferable that |β_{All}|-|β_{Dr}| ≥ 0.2°, |β_{All}|-|β_{Dr}| ≥ 0.5°, or |β_{All}|-|β_{Dr}| ≥ 1.0° is satisfied. This achieves further improvement in noise characteristics.

The upper limit of |β_{All}|-|β_{Dr}| is not particularly limited, and for example, |β_{All}|-|β_{Dr}| may be 5.0° or less, 4.0° or less, or 3.0° or less.

### (Relationship between |β_{All}|-|β_{Dr}| and σ_{All})

The grain-oriented electrical steel sheet 1 preferably satisfies |β_{All}|-|β_{Dr}| > σ_{All}/2. σ_{All} is the standard deviation of the absolute value of the β angle over the entire surface of the grain-oriented electrical steel sheet 1. There is variation in the β angle measured on the surface of the grain-oriented electrical steel sheet 1. An index of the variation of the β angle is σ_{All}. When |β_{All}|-|β_{Dr}| exceeds σ_{All}/2, it indicates that the region to be subjected to the magnetic domain control treatment is selectively determined by the β angle. Since the magnetic domain control treatment is performed in a concentrated manner in a region where the spacing of magnetic domain walls before the magnetic domain control is large and the iron loss reduction effect is large, the noise characteristics are further improved.

### (Relationship between σ_{Dr} and σ_{All})

The grain-oriented electrical steel sheet 1 preferably satisfies σ_{Dr} < σ_{All}. σ_{All} is the standard deviation of the absolute value of the β angle over the entire surface of the grain-oriented electrical steel sheet 1, and σ_{Dr} is the standard deviation of the absolute value of the β angle at the magnetic domain control points VP2, which are the intersection points of a plurality of the imaginary lines VL3 set at 2 mm intervals in parallel along the rolling direction RD of the grain-oriented electrical steel sheet 1 and the magnetic domain control treatment line 11. In the grain-oriented electrical steel sheet 1 satisfying σ_{Dr} < σ_{All}, the variation in β angle at the magnetic domain control point VP2 is smaller than the overall variation in β angle of the grain-oriented electrical steel sheet 1. That is, in this case, since the magnetic domain control treatment is intensively performed in a region where the spacing of magnetic domain walls before the magnetic domain control is large and the iron loss reduction effect is large, the noise characteristics are further improved.

### (Aspect of magnetic domain control treatment line 11)

The type of the magnetic domain control treatment line 11 is not particularly limited, but suitable examples thereof are the thermal strain and a groove. The thermal strain can be formed using means such as laser irradiation, electron beam irradiation, and ion implantation. The groove can be formed using means such as laser irradiation, electron beam irradiation, and machining.

The thermal strain disappears by the stress relief annealing or the heat treatment according thereto. Therefore, when the grain-oriented electrical steel sheet 1 is subjected to a heat treatment, the magnetic domain control treatment line 11 is preferably a groove. On the other hand, since the thermal strain can be easily formed, when simplification of a manufacturing step is required, it is preferable to set the magnetic domain control treatment line 11 to the thermal strain. The grain-oriented electrical steel sheet 1 may include both the thermal strain and groove.

Preferably, in the present embodiment, the magnetic domain control strength is determined according to the spacing of magnetic domain walls of the grain-oriented electrical steel sheet before the magnetic domain control treatment. The magnetic domain control strength means the amount of the thermal strain when the magnetic domain control means is a thermal strain, and means the depth of the groove when the magnetic domain control means is a groove.

The higher the strength of the magnetic domain control, the higher the effect of refining the magnetic domain. On the other hand, the higher the strength of magnetic domain control, the more easily the hysteresis loss is increased and the noise characteristics are deteriorated. According to the new findings of the present inventors, a grain-oriented electrical steel sheet has a non-uniform magnetic domain control saturation strength.

The magnetic domain control saturation strength is a magnetic domain control strength at which an effect of refining a magnetic domain is substantially saturated. When the magnetic domain control strength is equal to or lower than the magnetic domain control saturation strength, a higher magnetic domain control strength leads to reduced iron loss. However, when the magnetic domain control strength is more than the magnetic domain control saturation strength, the iron loss reduction effect is hardly enhanced even if the magnetic domain control strength is increased. On the other hand, even when the magnetic domain control strength is more than the magnetic domain control saturation strength, a higher magnetic domain control strength leads to increased hysteresis loss and worsened noise characteristics. Therefore, it is extremely preferable that the magnetic domain control strength is within the range not exceeding the magnetic domain control saturation strength.

In addition, the present inventors have found that the magnetic domain control saturation strength has a strong relationship with the β angle. In a point where the β angle is small, the magnetic domain control saturation strength is large. In the grain-oriented electrical steel sheet before the magnetic domain control treatment, there is a relationship also between the β angle and the spacing of magnetic domain walls. In the grain-oriented electrical steel sheet before the magnetic domain control treatment, the larger the β angle, the narrower the spacing of magnetic domain walls. However, in the grain-oriented electrical steel sheet after the magnetic domain control treatment, the relationship between the spacing of magnetic domain walls and the β angle becomes small. This is because the magnetic domain control treatment changes the spacing of magnetic domain walls, but does not change the β angle.

Therefore, it is preferable to select the optimum magnetic domain control strength according to the width of the spacing of magnetic domain walls or the β angle. Specifically, it is preferable that the magnetic domain control treatment is performed with a large magnetic domain control strength at a point where the spacing of magnetic domain walls is wide and the β angle is small; and the magnetic domain control treatment is performed with a low magnetic domain control strength at a point where the spacing of magnetic domain walls is narrow and the β angle is large. As described above, the magnetic domain control treatment is not performed on the region where the original spacing of magnetic domain walls is narrower than the predetermined value. As a result, a grain-oriented electrical steel sheet having non-uniform magnetic domain control strength is obtained. In such a grain-oriented electrical steel sheet, the iron loss of the grain-oriented electrical steel sheet after magnetic domain control is further reduced. On the other hand, in the grain-oriented electrical steel sheet after magnetic domain control, an increase in hysteresis loss and deterioration in noise characteristics are further suppressed.

FIG. 15 is a graph schematically illustrating a method for determining the magnetic domain control strength based on the spacing of magnetic domain walls. In FIG. 15, the vertical axis represents the magnetic domain control strength, and the horizontal axis represents the size of the spacing of magnetic domain walls. In FIG. 15, the solid line graph indicates the magnetic domain control saturation strength. In the region where the spacing of magnetic domain walls is narrow, the magnetic domain control effect cannot be obtained, and thus the magnetic domain control saturation strength is 0. For example, in a region where the spacing of magnetic domain walls exceeds 500 µm, the magnetic domain control effect is obtained. In the region where the spacing of magnetic domain walls exceeds 500 µm, as the spacing of magnetic domain walls increases, the magnetic domain control saturation strength also increases. For example, in a region where the spacing of magnetic domain walls exceeds about 1200 µm, the magnetic domain control saturation strength is substantially constant. Here, the region where the effect of the magnetic domain control is obtained is not limited to the region exceeding 500 µm. The region where the magnetic domain control saturation strength is substantially constant is not limited to a region exceeding about 1200 µm. These regions change depending on various conditions.

FIG. 16 shows a graph schematically illustrating a method for determining the magnetic domain control strength based on the β angle. In FIG. 16, the vertical axis represents the magnetic domain control strength, and the horizontal axis represents the magnitude of the β angle. A solid line graph in FIG. 16 indicates the magnetic domain control saturation strength. In the region where the β angle is large, the magnetic domain control effect cannot be obtained, and thus the magnetic domain control saturation strength is 0. In the region where the β angle is smaller than a predetermined value, the magnetic domain control effect is obtained. For example, it is estimated that the magnetic domain control effect can be obtained when the β angle is 2.0° or less. In the region where the β angle is smaller than a predetermined value, as the β angle increases, the magnetic domain control saturation strength also increases. In the region where the β angle is still smaller, the magnetic domain control saturation strength is substantially constant.

It is most preferable that the relationship between the spacing of magnetic domain walls of the point where the magnetic domain control is performed and the magnetic domain control strength is on the solid line graph in FIG. 11. Alternatively, it is most preferable that the relationship between the β angle of the point where the magnetic domain control is performed and the magnetic domain control strength is on the solid line graph in FIG. 16. The magnetic domain control saturation strength can be used as a target value of the magnetic domain control strength.

Furthermore, there is a magnetic domain control minimum strength, which is the minimum strength at which the magnetic domain control effect is exhibited. When the magnetic domain control is performed, the magnetic domain control strength is more preferably equal to or more than the magnetic domain control minimum strength.

However, the magnetic domain control strength may slightly vary with respect to the magnetic domain control saturation strength as a target value. In FIGS. 15 and 16, the region equal to or higher than the magnetic domain control minimum strength and within a certain range from the graph of the magnetic domain control saturation strength is referred to as a target range of the magnetic domain control strength. The magnetic domain control strength and the spacing of magnetic domain walls of the part to be subjected to the magnetic domain control are preferably within the shaded region surrounded by broken lines in FIGS. 15 and 16.

As a result, a grain-oriented electrical steel sheet having non-uniform magnetic domain control strength is obtained. In such a grain-oriented electrical steel sheet, the magnetic domain control strength varies depending on the β angle. In such a grain-oriented electrical steel sheet, the iron loss of the grain-oriented electrical steel sheet after magnetic domain control is further reduced. On the other hand, in the grain-oriented electrical steel sheet after magnetic domain control, an increase in hysteresis loss and deterioration in noise characteristics are further suppressed.

A plurality of the magnetic domain control treatment lines 11 provided on the surface of the grain-oriented electrical steel sheet 1 may be straight lines as illustrated in FIG. 1 or may be curved lines as illustrated in FIG. 14. When a plurality of the magnetic domain control treatment lines 11 provided on the surface of the grain-oriented electrical steel sheet 1 are curved, the degree of freedom of the magnetic domain control treatment is improved, so that it is easy to selectively perform the magnetic domain control treatment only on a portion having a small β angle, and the performance of the grain-oriented electrical steel sheet 1 is improved, which is preferable.

### (2. Manufacturing apparatus of grain-oriented electrical steel sheet 1)

Next, an example of a manufacturing apparatus of the grain-oriented electrical steel sheet 1 according to the present embodiment will be described. However, the manufacturing apparatus described below is merely exemplary. The grain-oriented electrical steel sheet 1 according to the present embodiment can be manufactured using an arbitrary device.

FIG. 6 illustrates an example of a hardware constitution of the image acquisition device 30 that acquires a magnetic domain image of the original sheet 2, that is, the grain-oriented electrical steel sheet 1 before the magnetic domain control treatment. The image acquisition device 30 includes a light source unit 31, a magneto-optical sensor (MO sensor 33), an image sensor 35, and a signal processing unit 37.

The light source unit 31 includes a light source including a light emitting diode (LED), and irradiates the MO sensor 33 with light having a uniform polarization plane.

The MO sensor 33 is a device that measures a magnetic domain structure of a magnetic material. The MO sensor 33 has an observed section on which a magnetic sample to be measured is placed. The light irradiated from the light source unit 31 passes through the inside of the MO sensor 33 and is reflected by the reflection layer. The reflected light passes through the inside of the MO sensor 33 again and is output to the outside of the MO sensor 33. When the original sheet 2 as a magnetic sample is placed on the observed section of the MO sensor 33, a leakage magnetic field corresponding to the direction of spontaneous magnetization of the original sheet 2 is generated inside the MO sensor 33. This leakage magnetic field rotates the polarization plane of the reflected light.

The image sensor 35 is a Complementary Metal-Oxide-Semiconductor (CMOS) image sensor. The image sensor 35 forms an image of the reflected light from the MO sensor 33 on the light receiving surface to perform photoelectric conversion, and outputs an analog signal after the photoelectric conversion to the signal processing unit 37. The distribution of the leakage magnetic field can be obtained by detecting the reflected light in which the polarization plane is rotated by the image sensor 35, and the magnetic domain structure of the original sheet 2 becomes clear.

The signal processing unit 37 includes an amplifier, an AD converter, a Digital Signal Processor (DSP), and the like. The analog signal output from the image sensor 35 is amplified by an amplifier. Then, the analog signal is converted into a digital signal by an AD converter. The digital signal is subjected to predetermined digital processing using a DSP to generate an image signal. The image signal generated by the signal processing unit 37 is output to the analysis device 40 (see FIG. 7) via a cable or by wireless communication.

FIG. 7 illustrates a hardware constitution of an analysis device 40 that analyzes the magnetic domain structure of the original sheet 2. The analysis device 40 is a computer device such as a personal computer (PC). The analysis device 40 includes a calculation unit 41, a memory 43, a display unit 45, an input unit 47, and a communication I/F 49.

The calculation unit 41 includes a Central Processing Unit (CPU). The calculation unit 41 analyzes the magnetic domain structure from the magnetic domain image of the original sheet 2 according to the program stored in the memory 43. Then, the calculation unit 41 determines a magnetic domain control treatment region 21 to which the magnetic domain control treatment is applied. The processing executed by the calculation unit 41 is described in detail later.

The memory 43 includes a Read Only Memory (ROM) and a Random Access Memory (RAM). The ROM stores programs executed by the CPU of the calculation unit 41 and data required for executing these programs. The program and data stored in the ROM are loaded into the RAM and executed.

The memory 43 may include a magnetic memory such as a hard disk drive (HDD) or an optical memory such as an optical disk. Alternatively, the memory 43 may be detachable from the analysis device 40 and store programs and data in a computer-readable recording medium. Alternatively, the memory 43 may receive the program executed by the calculation unit 41 from the network via the communication I/F 49.

The display unit 45 includes a display such as a liquid crystal display (LCD), a plasma display, or an organic electroluminescence (EL) display. The display unit 45 displays an image on the basis of the image signal output from the image acquisition device 30. In addition, the display unit 45 displays the analysis result of the magnetic domain structure by the calculation unit 41.

The input unit 47 includes an input device such as a mouse or a keyboard. The communication I/F 49 is an interface for transmitting and receiving data to and from an external device via a network such as a Local Area Network (LAN), a Wide Area Network (WAN), or the Internet.

Instead of general-purpose hardware such as a CPU, dedicated hardware specialized for analyzing a magnetic domain structure, such as an application specific integrated circuit (ASIC) or a Field Programmable Gate Array (FPGA), may be adopted as the calculation unit 41.

Note that FIGS. 6 and 7 illustrate a case where the image acquisition device 30 and the analysis device 40 are separate devices, but a system in which the image acquisition device 30 and the analysis device 40 are integrated may be adopted.

As means for introducing the thermal strain into the surface of the original sheet 2, known means such as laser irradiation, electron beam irradiation, and ion implantation can be adopted. As means for forming a groove on the surface of the original sheet 2, known means such as laser irradiation, electron beam irradiation, and machining can be adopted. Hereinafter, a constitution of the laser irradiation device 500 that introduces the thermal strain by laser irradiation will be described.

FIG. 8 illustrates a constitution of the laser irradiation device 500. The laser irradiation device 500 includes a polygon mirror 501, a light source device 503, a collimator 505, a condensing lens 507, a motor 509, a sensor 511, a control unit 513, and a sheet passing device 515.

The sheet passing device 515 passes the original sheet 2 in the rolling direction RD.

The polygon mirror 501 has, for example, a regular polygonal prism shape. A plurality of the plane mirrors is provided on each of a plurality of side surfaces constituting the polygon mirror 501 having a regular polygonal prism shape. The laser beam LB enters the plane mirror of the polygon mirror 501 in one direction (horizontal direction) from the light source device 503 via the collimator 505 and is reflected by the plane mirror.

The polygon mirror 501 is rotatable about the rotary shaft O1 by driving from the motor 509. The incident angle of the laser beam LB with respect to the plane mirror sequentially changes according to the rotation angle of the polygon mirror 501. As a result, the reflection direction of the laser beam LB is sequentially changed, and the surface of the original sheet 2 can be scanned. A Reference Number P in FIG. 8 represents an interval between the adjacent magnetic domain control treatment lines 11, that is, an irradiation pitch of the laser beam LB.

The light source device 503 outputs the laser beam LB by a predetermined irradiation system (for example, a continuous irradiation system or a pulse irradiation system) under the control of the control unit 513.

The condenser lens 507 is provided on the optical path of the laser beam LB reflected from the polygon mirror 501. The condenser lens 507 constitutes a condenser optical system having a predetermined focal distance. The laser beam LB reflected from the polygon mirror 501 is condensed on the surface of the original sheet 2 via the condenser lens 507, whereby the thermal strain is introduced into the surface of the original sheet 2.

The motor 509 is coupled to the polygon mirror 501. The motor 509 rotationally drives the polygon mirror 501 under the control of the control unit 513.

The sensor 511 is connected to a drive shaft of the motor 509. The sensor 511 detects a rotation angle of the polygon mirror 501 rotated by the motor 509. Furthermore, the sensor 511 outputs a signal (Hereinafter, the rotation angle signal is referred to as a rotation angle signal.) indicating the detected rotation angle to the control unit 513.

The control unit 513 includes a processor. The control unit 513 is connected to the light source device 503, the motor 509, the sensor 511, and the sheet passing device 515. The control unit 513 receives an input of a speed signal from the sheet passing device 515. Further, the control unit 513 outputs a signal instructing the motor 509 to rotationally drive the polygon mirror 501.

In addition, the control unit 513 controls on and off of the power of the laser beam LB output from the light source device 503 based on the stress introduction signal representing the magnetic domain control treatment region 21 and the rotation angle signal output from the sensor 511. When the laser irradiation device 500 is electrically connected to the analysis device 40, the stress introduction signal is input from the analysis device 40 to the laser irradiation device 500. The stress introduction signal may be input to the laser irradiation device 500 by an operator.

### (3. Method for manufacturing grain-oriented electrical steel sheet 1)

Next, a method for manufacturing the grain-oriented electrical steel sheet 1 according to the present embodiment will be described. According to the method for manufacturing a grain-oriented electrical steel sheet 1 according to the present embodiment, the grain-oriented electrical steel sheet 1 according to the present embodiment can be suitably manufactured. However, the manufacturing method described below is merely an example of a suitable manufacturing method of the grain-oriented electrical steel sheet 1, and does not limit the grain-oriented electrical steel sheet 1. For convenience of description, the manufacturing apparatus will be appropriately referred to in the description of the manufacturing method. However, the manufacturing apparatus mentioned below is merely a preferred example for carrying out the method for manufacturing the grain-oriented electrical steel sheet 1 according to the present embodiment.

As shown in the flowchart of FIG. 9, the method for manufacturing a grain-oriented electrical steel sheet 1 according to the present embodiment includes a step S62 of acquiring a magnetic domain image of an original sheet 2 of a grain-oriented electrical steel sheet 1, a step S64 of determining a magnetic domain control treatment region 21 based on distribution of the spacing of magnetic domain walls in the magnetic domain image, and a step S66 of applying the magnetic domain control treatment to the magnetic domain control treatment region 21 determined based on the distribution of the spacing of magnetic domain walls.

First, a magnetic domain image of the original sheet 2 is acquired (see S62 in FIG. 9). The original sheet 2 is the grain-oriented electrical steel sheet 1 before the magnetic domain control treatment is applied. The magnetic domain image can be acquired by, for example, the image acquisition device 30. Next, the distribution of the spacing of the 180° magnetic domain walls (spacing of magnetic domain walls) is derived from the magnetic domain image. The distribution of the spacing of magnetic domain walls in the original sheet 2 can be derived by using, for example, the calculation unit 41 of the analysis device 40.

Then, a region having a spacing of magnetic domain walls of a predetermined value or more (For example, about 500 µm or more) is determined as the magnetic domain control treatment region 21 (see S64 in FIG. 9). A region where the spacing of magnetic domain walls of the original sheet 2 is a predetermined value or more corresponds to a region 12A where the β angle is small in the grain-oriented electrical steel sheet 1.

The magnetic domain control treatment region 21 may be determined by visually observing the magnetic domain image displayed on the display unit 45 by the operator, and a stress introduction signal representing the magnetic domain control treatment region 21 may be input to the laser irradiation device 500.

Next, the magnetic domain control treatment is preferentially performed on the magnetic domain control treatment region 21 (see S66 in FIG. 9). Preferably, the magnetic domain control treatment is performed only on the magnetic domain control treatment region 21. When the magnetic domain control treatment line 11 is a thermal strain, the magnetic domain control treatment may be executed by irradiation of the laser beam LB by the laser irradiation device 500, or other means such as ion implantation or electron beam irradiation may be adopted. When the magnetic domain control treatment line 11 is a groove, the magnetic domain control treatment may be executed using a tool for machining.

An example of a method for determining the magnetic domain control treatment region 21 will be described in detail. The processing for specifying the magnetic domain control treatment region 21 is executed by, for example, the calculation unit 41 of the analysis device 40.

The calculation unit 41 derives the distribution of the spacing of magnetic domain walls of the original sheet 2 using, for example, a line segment method or Fourier transform. Then, the calculation unit 41 determines a region where the spacing of magnetic domain walls is a predetermined value or more (For example, about 500 µm or more) as a portion to which the magnetic domain control treatment is preferentially applied.

In the line segment method, evaluation is performed by drawing a line segment perpendicular to the magnetic domain. The line segments are drawn at intervals of three lines per 1 cm in a direction parallel to the magnetic domain. A spacing of magnetic domain walls is derived based on an interval between the intersection points of 180° magnetic domain walls and line segments.

The Fourier transform is particularly effective as a means for analyzing a magnetic domain structure of a magnetic body having a periodic magnetic domain structure such as the grain-oriented electrical steel sheet 1 and the original sheet 2. Hereinafter, a method for deriving a distribution of a spacing of magnetic domain walls of the original sheet 2 is described using a short-term two-dimensional Fourier transform (Hereinafter, it is referred to as "ST2DFT".) obtained by expanding a short-term Fourier transform, which is one of signal processing methods that have been used for time-frequency analysis of audio signals for a long time, to a two-dimensional region.

An image (magnetic domain image) represented by an image signal acquired by the image acquisition device 30 is expressed as x (k, 1) as a data column of two-dimensional coordinates (k-l coordinates). In the present embodiment, the magnetic domain image to be analyzed is an image binarized by two types of colors such as gray scale, or an image expressed by three or more gradations (multiple gradations).

In order to derive the distribution of the spacing of magnetic domain walls of the original sheet 2, the calculation unit 41 executes the following treatments of (A-1), (A-2), and (A-3).
(A-1) Treatment of cutting out a plurality of partial regions from magnetic domain image;
(A-2) Treatment of performing ST2DFT;
(A-3) Treatment of deriving distribution of spacing of magnetic domain walls.

Hereinafter, the treatment of A-1 to A-3 will be described in detail.

### (A-1) Treatment of cutting out a plurality of partial regions from magnetic domain image

In order to cut out a plurality of partial regions from a magnetic domain image and analyze each frequency structure, a window function Wa (k, 1) of a rectangular window in which a range in the k direction set to 0 ≤ k ≤ Nₖ-l and a range in the l direction set to 0 ≤ l ≤ Nₗ-1 is used (Nₖ and Nₗ are natural numbers). As the window function Wa (k, 1), a Hamming window, a Hanning window, a Blackman window, or the like can be applied.

When the observation position in the data column x (k, 1) of the magnetic domain image is expressed by an index (n, m), and the shift amounts of the window function Wa (k, l) in the k direction and the l direction are expressed as Sₖ and Sₗ, respectively (n, m, Sₖ, and Sₗ are integers.), a data column xₙₘ (k-nSₖ, l-mSₗ) of a partial region obtained by cutting out a range of nSₖ ≤ k ≤ nSₖ + Nₖ-1 and mSₗ ≤ 1 ≤ mSₗ + N₁-1 from the magnetic domain image is obtained as in Expression (1).
[Mathematical Formula 1] ${x}_{nm} \left(k-{nS}_{k},l-{mS}_{l}\right) = {W}_{a} \left(k-{nS}_{k},l-{mS}_{l}\right) x \left(k, l\right)$

FIG. 10 illustrates an example in which partial regions respectively corresponding to the observation positions (n, m) = (1, 1), (2, 2), (3, 3),..., and (P, Q) (P and Q are natural numbers) are cut out from the magnetic domain image G.

In the present embodiment, Nₖ and Nₗ that define the range of the window function Wa (k, 1) are parameters corresponding to the number of pixels in the k direction and the number of pixels in the l direction in the partial region, respectively.

### (A-2) Treatment of performing ST2DFT

When the data column of the partial region is defined as xₙₘ (n', m') = xₙₘ (k-nSₖ, l-mSₗ), and the two-dimensional Fourier transform is performed on xₙₘ (n', m'), a partial Fourier image X (fₖ, fₗ, n, m) corresponding to the partial region of the observation position (n, m) is obtained as in Expression (2).
[Mathematical Formula 2] $X \left({f}_{k}, {f}_{l}, n, m\right) = {\sum }_{n ′ = 0}^{{N}_{k} - 1} {\sum }_{m ′ = 0}^{{N}_{l} - 1} {x}_{nm} \left(n′,m′\right) exp \left\{-2πj\left(\frac{{f}_{k} n ′}{{N}_{k}}+\frac{{f}_{l} m ′}{{N}_{l}}\right)\right\}$

Here, fₖ and fₗ are space frequencies.

When the resolution of the space frequency fₖ is denoted by Δfₖ and the resolution of the space frequency fₗ is denoted by Δfₗ, Δfₖ and Δfₗ are defined as in Expression (3).
[Mathematical Formula 3] $\left\{\begin{matrix}Δ {f}_{k} = \frac{2}{{N}_{k} Δ k} \\ Δ {f}_{l} = \frac{2}{{N}_{l} Δ l}\end{matrix}\right.$

Δk and Δl are the space resolution in the k direction and the space resolution in the 1 direction in the magnetic domain image, respectively.

For example, when the two-dimensional Fourier transform is performed on the data column xₘₙ (k-nSₖ, l-mSₗ) of each partial region illustrated in FIG. 10, a partial Fourier image X (fₖ, fₗ, n, m) is obtained for each observation position (n, m) as illustrated in FIG. 11.

### (A-3) Treatment of deriving distribution of spacing of magnetic domain walls

When the partial Fourier image X (fₖ, fₗ, n, m) is obtained, the coordinates (k component fₖ^{max} (n, m) and l component fₗ^{max} (n, m)) of the peak position of the spot of the partial Fourier image X (fₖ, fₗ, n, m) are obtained. Note that, regarding the derivation of the peak position, a region in the vicinity of k = 0 and 1 = 0 is a part that greatly depends on the contrast of the image, and thus is excluded.

Then, the distribution L (n, m) of the spacing of magnetic domain walls is derived as in Expression (4) from the resolution of the space frequency defined by Expression (3) and the peak position of the spot of the partial Fourier image.
[Mathematical Formula 4] $L \left(n, m\right) = \frac{1}{\sqrt{{\left(Δ{f}_{k}{f}_{k}^{max}\left(n, m\right)\right)}^{2} + {\left(Δ{f}_{l}{f}_{l}^{max}\left(n, m\right)\right)}^{2}}}$

As described above, by using ST2DFT, it is possible to quantitatively derive the distribution L (n, m) of the spacing of magnetic domain walls while maintaining the position information of the magnetic domain image. FIGS. 4A to 4C described above illustrate the analysis result of the spacing of magnetic domain walls derived by ST2DFT.

FIG. 12 is a plan view of an example of the original sheet 2. FIG. 12 illustrates a magnetic domain control treatment region 21 and a non-magnetic domain control treatment region 22 of the original sheet 2 which are specified based on the magnetic domain image. The magnetic domain control treatment region 21 of the original sheet 2 substantially corresponds to a region 12A where the β angle is small in the grain-oriented electrical steel sheet 1. The non-magnetic domain control treatment region 22 of the original sheet 2 substantially corresponds to the region 12B where the β angle is large in the grain-oriented electrical steel sheet 1. The magnetic domain control treatment is applied to the broken line illustrated in FIG. 12.

When the calculation unit 41 derives the distribution L(n, m) of the spacing of magnetic domain walls, the calculation unit 41 determines the region where the spacing of magnetic domain walls are the predetermined value or more as the magnetic domain control treatment region 21 (that is, a region to which the magnetic domain control treatment is applied). The control unit 513 of the laser irradiation device 500 performs control to turn on the power of the laser beam LB with respect to the magnetic domain control treatment region 21, and preferably, to turn off the power of the laser beam LB with respect to the non-magnetic domain control treatment region 22 (that is, a region other than the magnetic domain control treatment region 21). As a result, the magnetic domain control treatment line 11 is introduced into the magnetic domain control treatment region 21 of the original sheet 2. Further, in the non-magnetic domain control treatment region 22 of the original sheet 2, introduction of the magnetic domain control treatment line 11 is suppressed to a minimum.

The magnetic domain image of the grain-oriented electrical steel sheet 1 after the magnetic domain control treatment can also be obtained by the above-described procedure. In the magnetic domain image of the grain-oriented electrical steel sheet 1, the magnetic domain control treatment line 11 may be unclear. In this case, the observation conditions may be adjusted so that the magnetic domain control treatment line 11 can be clearly confirmed. For example, the magnetic domain control treatment line 11 can be clarified by applying a DC magnetic field along the sheet surface perpendicular direction (thickness direction) of the grain-oriented electrical steel sheet 1.

Although embodiments of the present disclosure have been described above, the present disclosure is not limited thereto, and can be appropriately modified without departing from the technical idea. Hereinafter, a more preferable example of the grain-oriented electrical steel sheet 1 according to the present embodiment and the method for manufacturing the same will be described. Unless otherwise specified, the preferred aspect described below is applicable to both the grain-oriented electrical steel sheet 1 and the method for manufacturing the same. As described later, the grain-oriented electrical steel sheet according to the present embodiment may have a forsterite film and/or an insulating coating on the surface of the base steel sheet.

Each will be described below. However, when the grain-oriented electrical steel sheet includes a base steel sheet and a forsterite film and/or an insulating coating, the following regulations regarding the chemical composition, the magnetic domain control treatment line, the magnetic domain control region, and the non-magnetic domain control treatment line are regulations regarding the base steel sheet. However, the provision regarding the sheet thickness is a provision regarding the entire grain-oriented electrical steel sheet including the base steel sheet, and the forsterite film and/or the insulating coating.

### (Chemical composition and sheet thickness)

The chemical compositions of the grain-oriented electrical steel sheet 1 and the original sheet 2 are not limited as long as they are equivalent to those of the known grain-oriented electrical steel sheet 1. For example, the grain-oriented electrical steel sheet 1 and the original sheet 2 can contain, as a chemical composition, Si: 2.500 to 7.000%, Mn: 0.00 to 1.000%, C: 0 to 0.085%, acid-soluble Al: 0 to 0.065%, N: 0 to 0.012%, Cr: 0 to 0.300%, Cu: 0 to 0.400%, P: 0 to 0.500%, Sn: 0 to 0.300%, Sb: 0 to 0.300%, Ni: 0 to 1.000%, S: 0 to 0.015%, Se: 0 to 0.015%, Bi: 0 to 0.020%, Nb: 0 to 0.030%, V: 0 to 0.030%, Mo: 0 to 0.030%, Ta: 0 to 0.030%, W: 0 to 0.030%, B: 0 to 0.080%, and Ti: 0 to 0.015% in mass%. The balance of the chemical composition includes Fe and impurities.

The sheet thicknesses of the grain-oriented electrical steel sheet 1 and the original sheet 2 are not limited, but are preferably 0.15 to 0.30 mm, for example. When the thickness is 0.30 mm or less, classical eddy-current loss can be suppressed, and iron loss can be further improved. On the other hand, when the sheet thickness is 0.15 mm or more, rolling efficiency can be improved to improve productivity.

### (Surface treatment)

The grain-oriented electrical steel sheet 1 and the original sheet 2 may have a forsterite film. The grain-oriented electrical steel sheet 1 and the original sheet 2 may have an insulating coating. The forsterite film and the insulating coating may be formed on one surface or both surfaces of the grain-oriented electrical steel sheet 1.

The forsterite film is, for example, an inorganic coating film containing magnesium silicate as a main component. The forsterite film is formed, for example, by a reaction between an annealing separator containing magnesia (MgO) applied to the surface of the base steel sheet and a component of the surface of the base steel sheet in final annealing. The forsterite film has, for example, a composition (more specifically, a composition containing Mg₂SiO₄ as a main component) derived from the components of the annealing separator and the base steel sheet. On the other hand, when an annealing separator mainly containing Al₂O₃ is used in final annealing, a forsterite film may not be formed.

The insulating coating has a function of applying electrical insulation properties and tension to the grain-oriented electrical steel sheet 1. The tension is applied to the grain-oriented electrical steel sheet 1 to facilitate domain wall movement in the grain-oriented electrical steel sheet 1, and thus, the iron loss of the grain-oriented electrical steel sheet 1 can be reduced. In addition, according to the insulating coating, various characteristics such as corrosion resistance, heat resistance, and slippage can be provided to the grain-oriented electrical steel sheet 1. The insulating coating may be, for example, a known coating formed by applying a coating solution containing phosphate and colloidal silica as main components to the surface of the forsterite film and baking the coating solution.

The insulating coating is preferably formed after the final annealing and after the magnetic domain control treatment. On the other hand, the insulating coating may be formed after the final annealing step and before the magnetic domain control treatment. When the insulating coating is formed before the magnetic domain control treatment, the insulating coating may be peeled off in the magnetic domain control treatment line 11. Therefore, it is preferable to form the insulating coating again on the magnetic domain control treatment line 11 after the magnetic domain control treatment.

### (Angle formed by magnetic domain control treatment line 11 and transverse direction TD)

The angle formed by the magnetic domain control treatment line 11 and the transverse direction TD is not particularly limited. The magnetic domain control treatment line 11 and the transverse direction TD may be substantially parallel. That is, the angle formed by the magnetic domain control treatment line 11 and the transverse direction TD may be substantially 0°. On the other hand, as illustrated in FIG. 1, the angle formed by the magnetic domain control treatment line 11 and the transverse direction TD may be more than 0°. For example, the angle formed by the magnetic domain control treatment line 11 and the transverse direction TD may be an arbitrary value within the range of 0° to 45°. The angle formed by the magnetic domain control treatment line 11 and the transverse direction TD may be 1° or more, 3° or more, or 5° or more. The angle formed by the magnetic domain control treatment line 11 and the transverse direction TD may be 40° or less, 35° or less, or 30° or less.

As illustrated in FIG. 1, the angles formed by all the magnetic domain control treatment lines 11 and the transverse direction TD may be the same. That is, all the magnetic domain control treatment lines 11 may extend in parallel to each other. On the other hand, the angle formed by the magnetic domain control treatment line 11 and the transverse direction TD may vary. That is, some or all of a plurality of the magnetic domain control treatment lines 11 may extend non-parallel to each other. The average value of the angles formed by the magnetic domain control treatment line 11 and the transverse direction TD may be 1° or more, 3° or more, or 5° or more. The average value of the angles formed by the magnetic domain control treatment line 11 and the transverse direction TD may be 40° or less, 35° or less, or 30° or less. The average value of the angles may be calculated by measuring an angle formed with the transverse direction TD at a plurality of positions with respect to one magnetic domain control treatment line, or by measuring an angle formed with the transverse direction TD by a plurality of magnetic domain control treatment lines at one point or a plurality of positions.

### (Interval of magnetic domain control treatment line 11 along rolling direction RD)

The interval P along the rolling direction RD between the magnetic domain control treatment lines 11 adjacent along the rolling direction RD is not particularly limited. The effect of improving the iron loss is enhanced as the interval P is smaller. On the other hand, the larger the interval P, the more the noise characteristics are improved. The interval can be appropriately selected according to the characteristics required for the grain-oriented electrical steel sheet 1. For example, the interval P along the rolling direction RD between the magnetic domain control treatment lines 11 adjacent to each other along the rolling direction RD may be 1.0 mm or more, 2.0 mm or more, 3.0 mm or more, or 5.0 mm or more. The interval P along the rolling direction RD between the magnetic domain control treatment lines 11 adjacent along the rolling direction RD may be 10.0 mm or less, 9.0 mm or less, 8.0 mm or less, or 7.0 mm or less.

In the grain-oriented electrical steel sheet 1 exemplified in FIG. 1, the magnetic domain control treatment lines 11 are provided at regular intervals. On the other hand, the interval P along the rolling direction RD between the magnetic domain control treatment lines 11 adjacent along the rolling direction RD may vary. For example, the average value of the interval P along the rolling direction RD between the magnetic domain control treatment lines 11 adjacent to each other along the rolling direction RD may be 1.0 mm or more, 2.0 mm or more, 3.0 mm or more, or 5.0 mm or more. The average value of the intervals P along the rolling direction RD between the magnetic domain control treatment lines 11 adjacent along the rolling direction RD may be 10.0 mm or less, 9.0 mm or less, 8.0 mm or less, or 7.0 mm or less.

### (Magnitude of tensile stress introduced in thermal strain)

The magnetic domain control treatment line 11 may be due to a thermal strain. In the thermal strain, tensile stress is introduced. As the tensile stress is larger, the effect of improving the iron loss is enhanced. On the other hand, as the tensile stress is smaller, the noise characteristics are improved. Tensile stress according to characteristics required for the grain-oriented electrical steel sheet 1 can be appropriately selected.

The magnitude of the tensile stress is not particularly limited, but for example, in at least a part of the magnetic domain control treatment line 11, the tensile stress in an arbitrary direction is preferably 40 MPa or more, 60 MPa or more, or 80 MPa or more. When the tensile stress in at least one direction is 40 MPa or more, it is considered that the requirement that "the tensile stress in an arbitrary direction is 40 MPa or more" is satisfied. For example, in at least a part of the magnetic domain control treatment line 11, the tensile stress in an arbitrary direction is preferably 300 MPa or less, 200 MPa or less, 180 MPa or less, or 150 MPa or less. The tensile stress in an arbitrary direction in the magnetic domain control treatment line 11 may be uniform or may vary.

### (Depth and width of groove)

The magnetic domain control treatment line 11 may be a groove. As the depth and width of the groove are larger, the effect of improving the iron loss is enhanced. On the other hand, the noise characteristics are improved as the depth and width of the groove are smaller. The shape of the groove can be appropriately selected according to the characteristics required for the grain-oriented electrical steel sheet 1.

The depth of the groove is not particularly limited, but is preferably, for example, 5 µm to 50 µm. The depth of the groove may be 6 µm or more, 7 µm or more, or 10 µm or more. The depth of the groove may be 48 µm or less, 45 µm or less, or 40 µm or less.

The width of the groove is not particularly limited, but is preferably, for example, 10 µm to 300 µm. The width of the groove may be defined as 20 µm or more, 30 µm or more, or 50 µm or more. The width of the groove may be defined as 280 µm or less, 250 µm or less, or 200 µm or less. The depth and width of the groove may be uniform or may vary. In the case of variation, the average of the depths and widths of a plurality of the grooves is preferably in the above range.

### (Number of magnetic domain control points)

As the number of magnetic domain control points increases, the number of magnetic domain control treatment lines increases, and the region subjected to the magnetic domain control treatment increases. Therefore, from the viewpoint of iron loss reduction, it is preferable that the number of magnetic domain control points is large. For example, the number of magnetic domain control points in the grain-oriented electrical steel sheet 1 is preferably 10 points or more, 50 points or more, or 100 points or more per 10,000 mm².

### (Measurement method)

Hereinafter, a method for measuring various parameters of the grain-oriented electrical steel sheet 1 according to the present embodiment will be described. Note that measurement of any parameter is performed on a sample collected from the grain-oriented electrical steel sheet 1. For example, a rectangular sample having both sides of 100 mm (or 100 mm or more) in length can be cut out from the grain-oriented electrical steel sheet 1 and subjected to measurement. When the grain-oriented electrical steel sheet 1 is a coil, a sample may be collected from an arbitrary position of the coil. When the grain-oriented electrical steel sheet 1 is a component incorporated in an electrical product such as a transformer or a motor, a sample may be collected from any place of the component. When the size of the component is small, the length of one side of the sample may be less than 100 mm. In this case, the total value of the sample areas is set to 10,000 mm² or more. At that time, it is desirable to collect a sample by a method such as wire cutting in order to minimize the influence of mechanical strain or the like on the sample.

### (Method of identifying magnetic domain control treatment line 11)

When the magnetic domain control treatment line 11 is a groove, the magnetic domain control treatment line 11 can be visually identified. When the grain-oriented electrical steel sheet 1 has an insulating coating, the magnetic domain control treatment line 11 becomes visible by removing the insulating coating using a known peeling agent.

When the magnetic domain control treatment line 11 is a thermal strain, the magnetic domain control treatment line 11 may not be visually identified. In this case, for example, the magnetic domain image is photographed using the image acquisition device 30 as exemplified in FIG. 6. If necessary, a magnetic domain image is photographed while a DC magnetic field is applied along the rolling surface normal direction ND of the grain-oriented electrical steel sheet 1. The position of the thermal strain can be identified by observing the magnetic domain image.

### (Method for specifying rolling direction RD and transverse direction TD)

The rolling direction RD and the transverse direction TD of the grain-oriented electrical steel sheet 1 are specified by the following means.
(1) When the sample is cut out from the coil-shaped grain-oriented electrical steel sheet 1, the width direction of the coil is regarded as the transverse direction TD. A direction perpendicular to the transverse direction TD and the rolling surface normal direction ND is regarded as the rolling direction RD.
(2) When the sample is cut out from a part or the like of an electrical product, the rolling direction RD and the transverse direction TD are specified from rolling defects on the surface of the grain-oriented electrical steel sheet 1. The extending direction of the rolling defect is regarded as a rolling direction RD. A direction perpendicular to the rolling direction RD and the rolling surface normal direction ND is regarded as an transverse direction TD.
(3) When it is difficult to specify the rolling direction RD and the transverse direction TD from a rolling defect on the surface of the grain-oriented electrical steel sheet 1, the rolling direction RD and the transverse direction TD are specified from the crystal orientation of the grain-oriented electrical steel sheet 1. Specifically, the crystal orientation of the grain-oriented electrical steel sheet 1 to be evaluated is measured at a plurality of points. Then, the direction in which the deviation angle from the magnetization easy axis <001> at which the angle formed by the crystal orientation at the measurement point with the rolling surface normal direction ND (sheet thickness direction) is the closest to the right angle is minimized is regarded as the rolling direction RD, and the direction perpendicular to the rolling direction RD and the rolling surface normal direction ND is regarded as the transverse direction TD.

### (Method for measuring β angle)

The β angle is measured by the side surface reflection Laue method. The side surface reflection Laue method is widely known as a method for measuring a crystal orientation. However, the β angle is a value obtained by rounding off the measured numerical value to the second decimal place. That is, the significant digits of the β angle are up to the first decimal place.

### (Calculation method of |β_{All}|)

An outline of a method of calculating |β_{All}| is as follows. As illustrated in FIG. 13, measurement points are set in a grid pattern on the surface of a sample collected from the grain-oriented electrical steel sheet 1. The absolute value of the β angle is measured at each measurement point, and the average value thereof is calculated. This average value is regarded as |β_{All}|.

Specifically, an imaginary line VL1 parallel to the transverse direction TD and an imaginary line VL2 parallel to the rolling direction RD are set for the surface of the sample (rectangular region surrounded by alternate long and short dash line in FIG. 13) having one side of 100 mm or more. In setting the imaginary line VL1 and the imaginary line VL2, the presence of the magnetic domain control treatment line 11 is not considered. The interval between the imaginary lines VL1 is set to 2 mm. The interval between the imaginary lines VL2 is set to 2 mm. The imaginary line VL1 and the imaginary line VL2 are arranged over the entire surface of the sample. The absolute value of the β angle at the intersection point VP1 of the imaginary line VL1 and the imaginary line VL2 is measured.

### (Calculation method of |β_{Dr}|)

A method of calculating |β_{Dr}| is as follows. First, on the surface of a sample (rectangular region surrounded by alternate long and short dash line in FIG. 1 or 2) having a side of 100 mm or more, a plurality of the imaginary lines VL3 are set at regular intervals in parallel along the rolling direction RD of the grain-oriented electrical steel sheet 1. VL3 may be the same as or different from imaginary line VL2 parallel to rolling direction RD at the time of calculating |β_{All}|. The interval between the imaginary lines VL3 is 2 mm. The imaginary line VL3 is arranged over the entire surface of the sample. Next, the magnetic domain control point VP2 (that is, the intersection point of the imaginary line VL3 and the magnetic domain control treatment line 11) is specified. Then, the absolute value of the β angle at each magnetic domain control point VP2 is measured, and the average value thereof is calculated. This average value is regarded as |β_{Dr}|. The method of specifying the rolling direction RD and the magnetic domain control treatment line 11 and the method of measuring the β angle are as described above.

### (Method for measuring σ_{All})

σ_{All} is obtained by calculating the standard deviation of the absolute value of the β angle at each measurement point used to calculate |β_{All}|. The method for specifying the absolute value of the β angle at each measurement point is as described above.

### (Method for measuring σ_{Dr})

σ_{Dr} is obtained by calculating the standard deviation of the absolute value of the β angle at each magnetic domain control point VP2. The method for specifying the magnetic domain control point VP2 is as described above.

### (Method for measuring chemical components of original sheet 2 and grain-oriented electrical steel sheet 1)

The chemical compositions of the grain-oriented electrical steel sheet 1 and the original sheet 2 may be measured by a general analysis method of steel. For example, the chemical component may be measured using inductively coupled plasma-atomic emission spectrometry (ICP-AES). Specifically, the chemical composition of the grain-oriented electrical steel sheet 1 and the original sheet 2 can be measured by acquiring a test piece from the center portion in the thickness direction of the sample, and measuring the test piece under a condition based on a calibration curve prepared in advance using ICPS-8100 manufactured by Shimadzu Corporation or the like (measuring device). The contents of C and S, which are difficult to measure by ICP-AES, may be measured using a combustion-infrared light absorption method. The content of N may be measured using an inert gas fusion-thermal conductivity method.

When a forsterite film and/or an insulating coating are/is formed on the grain-oriented electrical steel sheet 1 and the original sheet 2, chemical components of the grain-oriented electrical steel sheet 1 and the original sheet 2 may be analyzed after removing the forsterite film and/or the insulating coating from the grain-oriented electrical steel sheet 1 and the original sheet 2.

The forsterite film can be removed, for example, by immersing the sample in sulfuric acid followed by immersion in nitric acid. Conditions such as the temperature and concentration of sulfuric acid and nitric acid and the time for immersion are appropriately adjusted so that the base metal of the sample is not excessively dissolved. An example of conditions of the removal operation of the forsterite film is as follows. First, the sample is immersed in sulfuric acid having a concentration of 10% at 80°C for 3 minutes. Thereafter, the surface of the sample is washed with water using a waste cloth or the like to remove the sludge adhering to the surface. Thereafter, the sample is dried. Further, the sample is immersed in nitric acid having a concentration of 10% at room temperature while being stirred for about 5 seconds.

The insulating coating can be removed, for example, by immersing the sample in a sodium hydroxide solution and then immersing the sample in dilute sulfuric acid and nitric acid. Conditions such as the temperature and concentration of sodium hydroxide, dilute sulfuric acid, and nitric acid solution, and the time for immersion are appropriately adjusted so that the base metal of the sample is not excessively dissolved. An example of the conditions of the removal operation of the insulating coating is as follows. First, the sample is immersed in a sodium hydroxide solution having a concentration of 20% at 80°C for 15 minutes. Thereafter, the sample is dried. Then, the sample is immersed in diluted sulfuric acid having a concentration of 10% at 80°C for 4 minutes. Thereafter, the sludge adhering to the surface of the sample is removed with a waste cloth or the like. Further, the sample is immersed in nitric acid having a concentration of 10% at room temperature while being stirred for about 10 seconds.

### (Method of measuring angle formed by magnetic domain control treatment line 11 and transverse direction TD)

The angle formed by the magnetic domain control treatment line 11 and the transverse direction TD can be measured using a known angle measuring means after the magnetic domain control treatment line 11 and the transverse direction TD are specified by the above-described procedure.

### (Method for measuring interval of magnetic domain control treatment line 11 along rolling direction RD)

The interval of the magnetic domain control treatment line 11 along the rolling direction RD can be measured using a known length measuring means after the magnetic domain control treatment line 11 and the rolling direction RD are specified by the above-described procedure.

### (Method for measuring magnitude of tensile stress introduced in thermal strain)

The magnitude of the tensile stress introduced in the thermal strain is measured by the EBSD Wilkinson method and Cross Court manufactured by BLG Vantage. The EBSD Wilkinson method is described in detail in A.J.Wilkinson, et al. "High-resolution elastic strain measurement from electron backscatter diffraction patterns: New levels of sensitivity" Ultramicroscopy Vol 106, No. 4-5, March 2006, P. 307-313.

When the magnitude of the tensile stress introduced in the thermal strain is measured by the EBSD Wilkinson method and the Cross Court manufactured by BLG Vantage, first, the magnetic domain control treatment line 11 is specified by the above-described procedure. Next, the grain-oriented electrical steel sheet 1 is cut through the magnetic domain control treatment line 11 and perpendicularly to the magnetic domain control treatment line 11. This cut cross section is used as a measurement surface. The cross section of the magnetic domain control treatment line 11 included in the measurement surface is analyzed by the EBSD Wilkinson method and Cross Court manufactured by BLG Vantage, and a tensile stress component in an arbitrary direction is extracted and the magnitude thereof is measured. For example, it is possible to extract a tensile stress component in a rolling surface normal direction ND, a direction parallel to the magnetic domain control treatment line 11, and a direction perpendicular to the rolling surface normal direction ND and the magnetic domain control treatment line 11.

The number of measurement points is, for example, 10. When the tensile stress in an arbitrary direction is 40 MPa or more (that is, when the tensile stress in at least one direction is 40 MPa or more,) in at least one location of the grain-oriented electrical steel sheet 1, the absolute maximum value of the tensile stress in an arbitrary direction in the magnetic domain control treatment line of the grain-oriented electrical steel sheet 1 is determined to be 40 MPa or more. Therefore, for the purpose of determining whether the absolute maximum value of the tensile stress is 40 MPa or more, the measurement of the tensile stress may be stopped when a measurement point at which the tensile stress in an arbitrary direction is 40 MPa or more is found. However, when σ(TSₘ)², TS_{m(β < 2)}, or TS_{m(β ≥ 2)} to be described later is obtained, the measurement is not stopped, and the tensile stress at each measurement point is obtained.

### (Method of measuring depth and width of groove)

The depth and width of the groove can be measured by specifying the surface shape of the sample using a known three-dimensional measuring machine. When the grain-oriented electrical steel sheet 1 has a tension insulation coating, the insulating coating is removed by the above-described procedure, and then the three-dimensional measurement of the sample surface is performed.

Preferably, in the grain-oriented electrical steel sheet according to the present embodiment, the magnetic domain control strength in the magnetic domain control treatment region is made non-uniform. The magnetic domain control strength means the absolute maximum value of tensile strength introduced into a thermal strain 541 when the magnetic domain control means is a thermal strain 541, and means the absolute maximum value of the depth of a groove 542 when the magnetic domain control means is a groove 542.

The "absolute maximum value of tensile strength introduced into a thermal strain 541" is the absolute maximum value of tensile strength measured in one arbitrary measurement cross section. It should be noted here that the magnitude and direction of tensile strength vary in one measurement cross section, and therefore one "absolute maximum value of tensile strength introduced into a thermal strain 541" is specified for one measurement cross section. As schematically illustrated in FIG. 17, the thermal strain 541 has a certain extent in the cross section. The tensile strength is largest at the point at which the laser is directly irradiates, and the tensile strength is small at the points away from the point. That is, the measured value of tensile strength differs for each measurement point and measurement direction in the cross section. According to the method for measuring tensile strength as described later, the distribution and the absolute maximum value of tensile strength in the cross section can be derived.

When the magnetic domain control strength is uniform, the absolute maximum value of tensile strength introduced into the thermal strain 541 is constant over the entire magnetic domain refinement treatment line 54. On the other hand, when the magnetic domain control strength is non-uniform, in the magnetic domain refinement treatment line, absolute maximum values of tensile strength introduced into the thermal strain are non-uniform at each measurement point of tensile strength. Hereinafter, the absolute maximum value of tensile strength introduced into a thermal strain may be simply referred to as "tensile strength".

The "absolute maximum value of the depth of a groove 542" is the absolute maximum value of the depth of a groove 542 at one arbitrary measurement point measured by a method described later. As schematically illustrated in FIG. 18, the depth of the groove 542 is also non-uniform at one measurement point. In general, the closer to the edge of the groove, the smaller the depth of the groove. Therefore, one "absolute maximum value of the depth of a groove 542" is specified for one measurement cross section.

When the magnetic domain control strength is uniform, the absolute maximum value of the depth of the groove 542 is constant over the entire magnetic domain refinement treatment line 54. On the other hand, when the magnetic domain control strength is non-uniform, in the magnetic domain refinement treatment line, absolute maximum values of the depth of the groove 542 are non-uniform at each measurement point of the depth of the groove. Hereinafter, the absolute maximum value of the depth of a groove 542 may be simply referred to as "the depth of a groove".

As described above, in a point where the β angle is small, the magnetic domain control saturation strength is large. It is preferable that a magnetic domain control treatment having high magnetic domain control strength is performed at a place where the β angle is small, and a magnetic domain control treatment having low magnetic domain control strength is performed at a place where the β angle is large. As described above, in the grain-oriented electrical steel sheet subjected to the magnetic domain control treatment for selecting the optimum magnetic domain control strength according to the magnitude of the β angle, the magnetic domain control strength in the magnetic domain control treatment region becomes non-uniform. In the magnetic domain control treatment line provided at a place where the β angle is large, the groove is shallow, or the tensile strength introduced into the thermal strain is small. In the magnetic domain control treatment line provided at a place where the β angle is small, the groove is deep, or the tensile strength introduced into the thermal strain is large. In such a grain-oriented electrical steel sheet, the iron loss of the grain-oriented electrical steel sheet after magnetic domain control is further reduced. On the other hand, in the grain-oriented electrical steel sheet after magnetic domain control, an increase in hysteresis loss and deterioration in noise characteristics are further suppressed.

When the magnetic domain control treatment line is a thermal strain, the grain-oriented electrical steel sheet preferably satisfies σ²(TSₘ) > 5.0. Here, TSₘ is the tensile strength in a unit of MPa introduced into the thermal strain measured at each of a plurality of the magnetic domain control points, which are the intersection points of a plurality of the imaginary lines VL3 and the magnetic domain control treatment line. σ²(TSₘ) is the variance of TSₘ.

When σ²(TSₘ) > 5.0 is satisfied, the magnetic domain control strength is changed based on the size of the spacing of magnetic domain walls or the magnitude of the β angle, and in the grain-oriented electrical steel sheet after magnetic domain control, an increase in hysteresis loss and deterioration in noise characteristics are further suppressed.

An example of a method of measuring TSₘ and σ²(TSₘ) is illustrated in FIG. 19. The broken line in FIG. 19 is the imaginary line VL3. An X mark and an O mark in FIG. 19 are intersection points of the imaginary line VL3 and the thermal strain 541 which is a magnetic domain control treatment line. The β angle is β_{Dr} or more at the point marked with the X mark, and the β angle is less than β_{Dr} at the point marked with the O mark. However, there is no need to consider the β angle at the intersection point for calculating σ²(TSₘ).

First, an intersection point of the imaginary line VL3 and the thermal strain 541 which is a magnetic domain control treatment line is specified. When the thermal strain 541 cannot be visually recognized with the naked eye, the thermal strain 541 is specified based on a magnetic domain image. The shape of the measurement region is preferably a rectangle having a size of 100 mm or more along the rolling direction RD and a size of 100 µm or more along the direction TD perpendicular to the rolling direction. One side of the rectangle is preferably parallel to the rolling direction RD.

Then, σm at all intersection points in the measurement region is measured, and the variance σ²(TSₘ) of σm is calculated.

The variance σ²(TS_{M}) of the absolute maximum values TS_{M} of tensile strength specified at each of a plurality of the measurement points is derived in accordance with the method for deriving a population variance described in the paragraph 2.36 of JIS Z 8101-1:2015 "Statistics-Vocabulary and symbols-Part 1: General statistical terms and terms used in probability".

Alternatively, when the magnetic domain control treatment line is a thermal strain, the grain-oriented electrical steel sheet preferably satisfies TS_{m(β < βDr)} > TS_{m(β} ≥ _{βDr)}. TS_{m(β < βDr)} is an arithmetical mean value of the absolute maximum value of the tensile strength in a unit of MPa introduced into the thermal strain, measured at each of the magnetic domain treatment points having the β angle of less than β_{Dr} among a plurality of the magnetic domain treatment points, which are the intersection points of a plurality of the imaginary lines VL3 set at intervals of 2 mm in parallel along the rolling direction of the grain-oriented electrical steel sheet and the magnetic domain control treatment line. TS_{m(β} ≥ _{βDr)} is an arithmetical mean value of the absolute maximum value of the tensile strength in a unit of MPa introduced into the thermal strain measured at each magnetic domain treatment point having a β angle of β_{Dr} or more.

When TS_{m(β < βDr)} > TS_{m(β} ≥ _{βDr)} is satisfied, the magnetic domain control strength is high at the place where the β angle is small, and the magnetic domain control strength is low at the place where the β angle is large. Therefore, the iron loss of the grain-oriented electrical steel sheet after magnetic domain control is further reduced. On the other hand, in the grain-oriented electrical steel sheet after magnetic domain control, an increase in hysteresis loss and deterioration in noise characteristics are further suppressed.

On the other hand, when the magnetic domain control treatment line is the groove 542, the grain-oriented electrical steel sheet preferably satisfies σ²(Dₘ) > 3.0. Dm is a depth of the groove 542 in a unit µm at a magnetic domain control point which is an intersection point of a plurality of the imaginary lines VL3 and the magnetic domain control treatment line. σ²(Dₘ) is a variance of Dₘ.

When σ²(Dₘ) > 3.0 is satisfied, the magnetic domain control strength is changed based on the size of the spacing of magnetic domain walls or the magnitude of the β angle, and in the grain-oriented electrical steel sheet after magnetic domain control, an increase in hysteresis loss and deterioration in noise characteristics are further suppressed.

An example of a method for measuring Dₘ and σ²(Dₘ) is illustrated in FIG. 20. In FIG. 20, the broken lines represent a plurality of the imaginary lines VL3 set at intervals of 2 mm in parallel along the rolling direction RD of the grain-oriented electrical steel sheet. An X mark and an O mark in FIG. 20 are intersection points of the imaginary lines VL3 and the groove 542 which are the magnetic domain control treatment lines. The β angle is β_{Dr} or more at the point marked with the X mark, and the β angle is less than β_{Dr} at the point marked with the O mark. However, there is no need to consider the β angle at the intersection point for calculating σ²(Dₘ).

First, an intersection point of the imaginary line VL3 and the magnetic domain control treatment line is specified. When the magnetic domain control treatment line cannot be visually recognized with the naked eye, the magnetic domain control treatment line is specified based on the magnetic domain image. When the magnetic domain refinement treatment line is a groove 542, it is easy to visually recognize the magnetic domain refinement treatment line with the naked eye. The shape of the measurement region is preferably a rectangle having a size of 100 mm or more along the rolling direction RD and a size of 100 mm or more along the direction TD perpendicular to the rolling direction. One side of the rectangle is preferably parallel to the rolling direction RD.

Then, the absolute maximum value Dₘ of the depth of the groove is measured for all the intersection points in the measurement region, and the variance σ²(Dₘ) of the absolute maximum value Dₘ of the depth of the groove is calculated. A method of measuring the maximum depth Dm of the groove is as follows. Measurement is performed using a white interference microscope Contour GT-I manufactured by Bruker. As the lenses to be used, an objective lens of 5 times (numerical aperture: 0.12, optical resolution: 2.2 µm) and an inner lens of 1 time are used, and a white LED is used as the light source and a monochrome CCD (1200 × 1000 pixels) is used as the camera. The pixel size was 1.37 µm, inclination correction was performed by fitting to the least-square plane using analysis software Vision64 Map Premium9.2, and then undulation of long wavelength was removed using a Gaussian filter with a cutoff value of 2.5 mm for analysis. Note that resampling may be performed so that the pixel size is 10 µm as necessary at the time of analysis. In addition, a portion that is obviously determined to be an abnormal point may be excluded from the analysis, and the type of the lens, the value of the filter, and the correction method may be changed depending on the properties of the sample. When a groove is formed in the grain-oriented electrical steel sheet but the unevenness cannot be measured from the surface due to an insulating coating or the like, the measurement is performed after the insulating coating or the like is removed using a known method.

Alternatively, when the magnetic domain control treatment line is the groove 542, the grain-oriented electrical steel sheet preferably satisfies D_{m(β < βDr)} > D_{m(β≥ βDr)}. D_{m(β < βDr)} is an arithmetical mean value of the absolute maximum value of the groove depth in a unit of µm measured at each of the magnetic domain control points having the β angle of less than β_{Dr} among a plurality of the magnetic domain control points, which are the intersection points of a plurality of the imaginary lines VL3 set at intervals of 2 mm in parallel along the rolling direction of the grain-oriented electrical steel sheet, and the magnetic domain control treatment line. D_{m(β ≥ βDr)} is an arithmetical mean value of the absolute maximum values of the depth of the groove in a unit of µm, the maximum values being measured at each of the magnetic domain control points having the β angle of β_{Dr} or more.

In the magnetic domain control treatment line satisfying the formula, the magnetic domain control strength is high at the place where the β angle is small, and the magnetic domain control strength islow at the place where the β angle is large. Therefore, the iron loss of the grain-oriented electrical steel sheet after magnetic domain control is further reduced. On the other hand, in the grain-oriented electrical steel sheet after magnetic domain control, an increase in hysteresis loss and deterioration in noise characteristics are further suppressed.

An example of a method for measuring TSₘ(β < 2) and TSₘ(β ≥ 2) is illustrated in FIG. 20. As described above, the X mark and the O mark in FIG. 20 are the intersection points of the imaginary line VL3 and the grooves 542 which are the magnetic domain control treatment lines. The β angle at the portion marked with X is β_{Dr} or more, and the β angle at the portion marked with O is less than β_{Dr}.

First, the β angle is measured at each intersection to specify the intersection points where the β angle is β_{Dr} or more and the intersection points where the β angle is less than β_{Dr}. Next, an arithmetical mean value of Dₘ at all intersection points where the β angle is β_{Dr} or more is calculated, and this is regarded as D_{m(β≥βDr)}. Furthermore, the arithmetical mean value of Dₘ at all intersection points where the β angle is less than β_{Dr} is calculated, and this is regarded as D_{m(β≥βDr)}. The method for measuring the absolute maximum value Dₘ of the depth of the groove at the intersection point is as described above.

### Examples

The effect of an aspect of the present disclosure will be described more specifically with reference to Examples. However, the conditions in Examples are merely one condition example adopted to confirm the enablement and effects of the present disclosure. The present disclosure is not limited to this one condition example. The present disclosure can adopt various conditions as long as the object of the present disclosure is achieved without departing from the gist of the present disclosure.

### (First Example)

Grain-oriented electrical steel sheets in the same lot having a sheet thickness of 0.23 mm and classified into 23P085 in the table 2 of JIS C 2553:2019 "Cold-rolled grain-oriented electrical steel strip and sheet delivered in the fully-processed state" were used as original sheets. The original sheet was subjected to a magnetic domain control treatment under various conditions shown in Table 1. The noise and iron loss of the grain-oriented electrical steel sheets subjected to the magnetic domain control treatment obtained as a result are evaluated and described in Table 2. In Table 1, values outside the range of the grain-oriented electrical steel sheet according to the present embodiment are underlined. In Table 2, values that do not satisfy the following pass/fail criteria are underlined.

The evaluation methods for the noise and the transformer iron loss W15/60 were as follows. Hereinafter, the transformer iron loss W15/60 is simply referred to as an iron loss. First, 180 grain-oriented electrical steel sheets having a sheet thickness of 0.23 mm were laminated to form a three-phase transformer core. The widths of the foot and the yoke of the three-phase transformer core were both 150 mm. The height and width of the outer shape of the three-phase transformer core were both 750 mm. Noise and iron loss of these three-phase transformer cores were measured. The measurement conditions were a frequency of 60 Hz and an excitation magnetic flux density of 1.5 T.

In measuring the noise, microphones were arranged at equal intervals at eight points around the transformer in which the three-phase transformer core was incorporated. The distance between the transformer and the microphone was 30 cm. The values obtained by correcting the A characteristics to the noise measurement results by the microphones and averaging the results are described in Table 2 as the noise evaluation results (unit: dBA) of the grain-oriented electrical steel sheets. An example in which the evaluation result of noise was 30.50 dBA or less was determined to be an example in which noise reduction was achieved. The noise evaluation result determined to be unacceptable was underlined.

The iron loss was obtained by measuring voltages and currents on the primary side and the secondary side with a power analyzer when excitation was performed at a frequency of 60 Hz and an excitation magnetic flux density of 1.5 T as described above. The determined iron loss is described in Table 2 as an iron loss evaluation result (unit: W/kg) of the three-phase transformer. An example in which the evaluation result of the iron loss was 0.850 W/kg or less was determined to be an example in which iron loss reduction was achieved. The noise evaluation result determined to be unacceptable was underlined.

Further, |β_{All}|, |β_{Dr}|, σ_{All}, and σ_{Dr} in the grain-oriented electrical steel sheets subjected to the magnetic domain control treatment were measured and described in Table 2. The measurement method was in principle according to the procedure described above. A rectangular sample having both sides of 100 mm in length was cut out from a three-phase transformer core for measuring noise and iron loss, and subjected to measurement.

**[Table 1]**

| Example No. | \|β_{All}\|-\|β_{Dr}\| | σ_{All} | σ_{Dr} | Type of magnetic domain control treatment line | Remarks |
|---|---|---|---|---|---|
| 1 | 0.1 | 1.5 | 1.6 | Thermal strain | Treatment line in region where the β angle is small |
| 2 | 0.1 | 1.5 | 1.6 | Groove | Treatment line in region where the β angle is small |
| 3 | 0.1 | 1.5 | 1.6 | Mixed | Treatment line in region where the β angle is small |
| 4 | 0.4 | 1.2 | 1.3 | Thermal strain | Treatment line in region where the β angle is small |
| 5 | 0.6 | 1.2 | 1.2 | Thermal strain | Treatment line in region where the β angle is small |
| 6 | 1.1 | 1.2 | 1.2 | Thermal strain | Treatment line in region where the β angle is small |
| 7 | 2.7 | 1.5 | 1.5 | Thermal strain | Treatment line in region where the β angle is small |
| 8 | 1.3 | 0.8 | 1.0 | Thermal strain | Treatment line in region where the β angle is small |
| 9 | 1.2 | 1.4 | 0.8 | Thermal strain | Treatment line in region where the β angle is small |
| 10 | 0.0 | 1.5 | 1.5 | Thermal strain | straight line treatment line over the entire width |
| 11 | 0.0 | 1.4 | 1.4 | Thermal strain | Random broken-line treatment line |
| 12 | 0.0 | 1.3 | 1.3 | Thermal strain | Regular dashed-line treatment line |
| 13 | -0.5 | 1.2 | 1.3 | Thermal strain | Treatment line in region where the β angle is large |
| 14 | -1.1 | 1.2 | 1.2 | Thermal strain | Treatment line in region where the β angle is large |

**[Table 2]**

| Example No. | Evaluation results of noise | Evaluation results of iron loss |
|---|---|---|
| 1 | 30.20 | 0.830 |
| 2 | 29.80 | 0.847 |
| 3 | 30.00 | 0.837 |
| 4 | 27.70 | 0.836 |
| 5 | 26.00 | 0.839 |
| 6 | 25.60 | 0.845 |
| 7 | 25.40 | 0.848 |
| 8 | 24.90 | 0.845 |
| 9 | 24.80 | 0.845 |
| 10 | 33.60 | 0.831 |
| 11 | 33.05 | 0.850 |
| 12 | 32.94 | 0.852 |
| 13 | 29.20 | 0.865 |
| 14 | 25.20 | 0.866 |

In Example No. 10, all the magnetic domain control treatment lines were formed over the entire width of the grain-oriented electrical steel sheet. As a result, Example No. 10 did not satisfy |β_{All}|-|β_{Dr}| ≥ 0.1°. In Example No. 10, the iron loss was within the acceptable range, but the noise characteristics were unacceptable.

In Example No. 11, the magnetic domain control treatment line was formed in a broken line shape. That is, in Example No. 11, similarly to Example No. 1 to 9, a region where the magnetic domain control treatment is not performed is provided. However, in Example No. 11, the sizes of the gaps between the magnetic domain control treatment lines included in the broken line were randomly varied. Portions where the magnetic domain control treatment was not performed were randomly provided without considering the distribution of the spacing of magnetic domain walls in the magnetic domain image at all. As a result, Example No. 11 did not satisfy |B_{All}|-|_{βDr}| ≥ 0.1°. In Example No. 11, the iron loss was within the acceptable range, but was the same value as 0.850 which is the determination value of acceptance. In addition, in Example No. 11, the noise characteristics were unacceptable.

In Example No. 12, the magnetic domain control treatment lines were formed in an ordered broken line shape. That is, in Example No. 12, similarly to Example No. 1 to 9, a region where the magnetic domain control treatment is not performed is provided. However, in Example No. 12, the size of the gap between the magnetic domain control treatment lines included in the broken line is set to a constant value. Portions where the magnetic domain control treatment was not performed were regularly provided without considering the distribution of the spacing of magnetic domain walls in the magnetic domain image at all. As a result, Example No. 12 did not satisfy |β_{All}|-|β_{Dr}| ≥ 0.1°. In Example No. 12, both the iron loss and the noise characteristic were unacceptable.

In Example No. 13 and Example No. 14, the magnetic domain control treatment was intentionally applied to a region where the β angle is large. These examples also did not satisfy |β_{All}| -|β_{Dr}| ≥ 0.1°. In Example No. 13 and Example No. 14, the iron loss was unacceptable.

On the other hand, in Example No. 1 to 9, the magnetic domain control treatment was applied to a magnetic domain control treatment region (region having a small β angle) limited based on the distribution of the spacing of magnetic domain walls. Example No. 1 to 9 satisfied |β_{All}|-|β_{Dr}| ≥ 0.1°, and both the noise characteristics and the iron loss fell within the acceptable range. By Examples Nos. 1 to 9, both iron loss reduction and noise reduction were achieved.

By Examples Nos. 1 to 9, it was confirmed that the larger |β_{All}|-|β_{Dr}|, the better the noise characteristics. In Example No. 6 to 9, |β_{All}|-|β_{Dr}| > σ_{All}/2 was satisfied. In Example 9, σ_{Dr} < σ_{All} was satisfied. In these examples, the noise characteristics and the iron loss were further excellent.

### (Second Example)

In order to evaluate the characteristics of the grain-oriented electrical steel sheet having a non-uniform magnetic domain control strength, experiments described below were conducted. In all the examples, |β_{All}|-|β_{Dr}| ≥ 0.1° was satisfied.

Magnetic domain control treatment was performed on the original sheet under various conditions. The noise and iron loss of the grain-oriented electrical steel sheets subjected to the magnetic domain control treatment obtained as a result were evaluated and described in Tables 3 and 4 together with the conditions. As the original sheet, a grain-oriented electrical steel sheet having a sheet thickness of 0.23 mm and classified into 23P085 in the table 2 of JIS C 2553:2019 "Cold-rolled grain-oriented electrical steel strip and sheet delivered in the fully-processed state" was used.

The method for measuring noise and iron loss and the evaluation method were the same as those in Example 1.

**[Table 3]**

| Example No. | σ² (TSₘ) | TSₘ (β < β_{Dr}) | TSₘ (β ≥ β_{Dr}) | \|β_{All}\|-\|β_{Dr}\| | σ_{All} | O_{Dr} | Evaluation results of noise | Evaluation results of iron loss |
|---|---|---|---|---|---|---|---|---|
| A1 | 0.2 | 148 | 151 | 0.1 | 0.5 | 0.7 | 30.26 | 0.830 |
| A2 | 2.3 | 151 | 153 | 0.2 | 0.5 | 0.7 | 24.35 | 0.820 |
| A3 | 5.1 | 147 | 162 | 0.2 | 0.5 | 0.7 | 24.24 | 0.807 |
| A4 | 2.7 | 181 | 123 | 0.2 | 0.5 | 0.7 | 22.73 | 0.820 |
| A5 | 5.1 | 175 | 111 | 0.2 | 0.5 | 0.7 | 22.75 | 0.805 |
| A6 | 3.1 | 152 | 153 | 0.2 | 0.3 | 0.5 | 23.83 | 0.814 |
| A7 | 5.3 | 149 | 158 | 0.3 | 0.4 | 0.5 | 23.75 | 0.801 |
| A8 | 2.6 | 176 | 141 | 0.3 | 0.4 | 0.5 | 22.84 | 0.813 |
| A9 | 5.1 | 198 | 150 | 0.3 | 0.4 | 0.5 | 22.32 | 0.800 |
| A10 | 3.2 | 155 | 157 | 0.2 | 0.5 | 0.4 | 23.43 | 0.819 |
| A11 | 5.1 | 148 | 159 | 0.3 | 0.7 | 0.5 | 23.42 | 0.807 |
| A12 | 2.8 | 181 | 132 | 0.3 | 0.7 | 0.5 | 22.21 | 0.820 |
| A13 | 5.2 | 198 | 155 | 0.3 | 0.7 | 0.5 | 21.98 | 0.807 |
| A14 | 5.5 | 204 | 148 | 0.5 | 0.4 | 0.3 | 21.55 | 0.797 |

Example No. A1 satisfied |β_{All}|-|β_{Dr}| ≥ 0.1, and thus showed better iron loss evaluation results and noise evaluation results than the conventional grain-oriented electrical steel sheet.

On the other hand, in Example No. A2, in addition to satisfying |β_{All}|-|β_{Dr}| ≥ 0.1, the absolute maximum value of the tensile strength introduced to the amount of the thermal strain in the magnetic domain control treatment line was non-uniform at each measurement point of the tensile strength. The evaluation results of iron loss and noise of Example No. A2 were further superior to those of Example No. A1.

In Example No. A3, in addition to satisfying |β_{All}|-|β_{Dr}| ≥ 0.1, the absolute maximum value of the tensile strength introduced to the amount of the thermal strain in the magnetic domain control treatment line was non-uniform at each measurement point of the tensile strength, and σ²(TSₘ) > 5.0 was further satisfied. The evaluation results of iron loss and noise of Example No. A3 were further superior to those of Example Nos. A1 and A2.

In Example No. A4, in addition to satisfying |β_{All}|-|β_{Dr}| ≥ 0.1, the absolute maximum value of the tensile strength introduced to the amount of the thermal strain in the magnetic domain control treatment line was non-uniform at each measurement point of the tensile strength, and TS_{m(β < βDr)} > TS_{m(β ≥ βDr)} was further satisfied. At least one of the evaluation results of the iron loss and the noise of Example No. A4 was more excellent than those of Example Nos. A1 and A2.

In Example No. A5, in addition to satisfying |β_{All}|-|β_{Dr}| ≥ 0.1, the absolute maximum value of the tensile strength introduced to the amount of the thermal strain in the magnetic domain control treatment line was non-uniform at each measurement point of the tensile strength, and σ²(TSₘ) > 5.0 and TS_{m(β< βDr)} > TS_{m(β≥βDr)} was further satisfied. At least one of the evaluation results of the iron loss and the noise of Example No. A5 was more excellent than those of Example Nos. A1 to A5.

In Example No. A6, in addition to satisfying |β_{All}|-|β_{Dr}| ≥ 0.1, the absolute maximum value of the tensile strength introduced to the amount of the thermal strain in the magnetic domain control treatment line was non-uniform at each measurement point of the tensile strength, and |β_{All}|-|β_{Dr}| > σ_{All}/2 was satisfied. The evaluation results of iron loss and noise of Example No. A6 were further superior to those of Example Nos. A1 and A2.

In Example No. A7, in addition to satisfying |β_{All}|-|β_{Dr}| ≥ 0.1, the absolute maximum value of the tensile strength introduced to the amount of the thermal strain in the magnetic domain control treatment line was non-uniform at each measurement point of the tensile strength, and |β_{All}|-|β_{Dr}| > σ_{All}/2 was satisfied in addition to satisfying σ²(TSₘ) > 5.0. The evaluation results of iron loss and noise of Example No. A7 were further superior to those of Example Nos. A1 to A3 and A6.

In Example No. A8, in addition to satisfying |β_{All}| -|β_{Dr}| ≥ 0.1°, the absolute maximum value of the tensile strength introduced to the amount of the thermal strain in the magnetic domain control treatment line was non-uniform at each measurement point of the tensile strength, and |β_{All}|-|β_{Dr}| > σ_{All}/2 was satisfied in addition to satisfying TS_{m(β < βDr)} > TS_{m(β ≥ βDr)}. At least one of the evaluation results of the iron loss and the noise of Example No. A8 was more excellent than those of Example Nos. A1 to A4 and A6.

In Example No. A9, in addition to satisfying |β_{All}|-|β_{Dr}| ≥ 0.1°, the absolute maximum value of the tensile strength introduced to the amount of the thermal strain in the magnetic domain control treatment line was non-uniform at each measurement point of the tensile strength, and |β_{All}|-|β_{Dr}| > σ_{All}/2 was satisfied in addition to satisfying σ²(TSₘ) > 5.0 and TS_{m(β< βDr)} > TS_{m(β≥βDr)}. The evaluation results of iron loss and noise of Example No. A9 were further superior to those of Examples Nos. A1 to A5 and A6 to A8.

In Example No. A10, in addition to satisfying |β_{All}|-|β_{Dr}| ≥ 0.1, the absolute maximum value of the tensile strength introduced to the amount of thermal strain in the magnetic domain control treatment line was non-uniform at each measurement point of the tensile strength, and σ_{Dr} < σ_{All} was satisfied. The evaluation results of iron loss and noise of Example No. A10 were further superior to those of Example Nos. A1 and A2.

In Example No. A11, in addition to satisfying |β_{All}|-|β_{Dr}| ≥ 0.1, the absolute maximum value of the tensile strength introduced to the amount of the thermal strain in the magnetic domain control treatment line was non-uniform at each measurement point of the tensile strength, and α_{Dr} < σ_{All} was satisfied in addition to satisfying σ²(TSₘ) > 5.0. At least one of the evaluation results of the iron loss and the noise of Example No. A11 was more excellent than those of Example Nos. A1 to A3 and A10.

In Example No. A12, in addition to satisfying |β_{All}|-|β_{Dr}| ≥ 0.1°, the absolute maximum value of the tensile strength introduced to the amount of the thermal strain in the magnetic domain control treatment line was non-uniform for each measurement point of the tensile strength, and σ_{Dr} < σ_{All} was satisfied in addition to satisfying TS_{m(β< βDr)} > TS_{m(β≥ βDr)}. At least one of the evaluation results of the iron loss and the noise of Example No. A12 was more excellent than those of Example Nos. A1 to A4 and A10.

In Example No. A13, in addition to satisfying |β_{All}|-|β_{Dr}| ≥ 0.1°, the absolute maximum value of the tensile strength introduced to the amount of the thermal strain in the magnetic domain control treatment line was non-uniform for each measurement point of the tensile strength, and σ_{Dr} < σ_{All} was satisfied in addition to satisfying σ²(TSₘ) > 5.0 and TS_{m(β < βDr)} > TS_{m(β ≥ βDr)}. At least one of the evaluation results of the iron loss and the noise of Example No. A13 was more excellent than those of Examples Nos. A1 to A5 and A10 to A12.

In Example No. A14, in addition to satisfying |β_{All}|-|β_{Dr}| ≥ 0.1°, the absolute maximum value of the tensile strength introduced to the amount of the thermal strain in the magnetic domain control treatment line was non-uniform for each measurement point of the tensile strength, and |β_{All}|-|β_{Dr}| > σ_{All}/2 and σ_{Dr} < σ_{All} were satisfied in addition to satisfying σ²(TSₘ) > 5.0 and TS_{m(β < βDr)} > TS_{m(β ≥ βDr)}. The evaluation results of iron loss and noise of Example No. A14 were the best among those of Example Nos. A1 to A14.

**[Table 4]**

| Example No. | σ² (Dₘ) | Dₘ (β < β_{Dr}) | Dₘ (β ≥ β_{Dr}) | \|β_{All}\|-\|β_{Dr}\| | σ_{All} | σ_{Dr} | Evaluation results of noise | Evaluation results of iron loss |
|---|---|---|---|---|---|---|---|---|
| B1 | 0.3 | 25 | 25 | 0.1 | 0.5 | 0.7 | 30.07 | 0.831 |
| B2 | 1.2 | 25 | 31 | 0.2 | 0.5 | 0.7 | 24.14 | 0.823 |
| B3 | 3.4 | 28 | 32 | 0.2 | 0.5 | 0.7 | 24.06 | 0.809 |
| B4 | 1.8 | 35 | 28 | 0.2 | 0.5 | 0.7 | 22.53 | 0.821 |
| B5 | 3.4 | 31 | 22 | 0.2 | 0.5 | 0.7 | 22.52 | 0.808 |
| B6 | 1.6 | 28 | 29 | 0.2 | 0.3 | 0.5 | 23.64 | 0.817 |
| B7 | 3.3 | 26 | 38 | 0.3 | 0.4 | 0.5 | 23.54 | 0.802 |
| B8 | 2.7 | 35 | 15 | 0.3 | 0.4 | 0.5 | 22.64 | 0.814 |
| B9 | 3.1 | 27 | 18 | 0.3 | 0.4 | 0.5 | 22.21 | 0.803 |
| B10 | 2.1 | 27 | 30 | 0.2 | 0.5 | 0.4 | 23.22 | 0.822 |
| B11 | 3.4 | 28 | 38 | 0.3 | 0.7 | 0.5 | 23.22 | 0.809 |
| B12 | 1.9 | 30 | 18 | 0.3 | 0.7 | 0.5 | 22.02 | 0.821 |
| B13 | 3.2 | 28 | 25 | 0.3 | 0.7 | 0.5 | 21.78 | 0.809 |
| B14 | 3.6 | 36 | 10 | 0.5 | 0.4 | 0.3 | 21.37 | 0.798 |

Example No. B1 satisfied |β_{All}|-|β_{Dr}| ≥ 0.1°, and thus showed better iron loss evaluation results and noise evaluation results than the conventional grain-oriented electrical steel sheet.

In Example No. B2, in addition to satisfying |β_{All}|-|β_{Dr}| ≥ 0.1°, the absolute maximum value of the depth of the groove in the magnetic domain control treatment line was non-uniform for each measurement point of the groove. The evaluation results of iron loss and noise of Example No. B2 were further superior to those of Example No. B1.

In Example No. B3, in addition to satisfying |β_{All}|-|β_{Dr}| ≥ 0.1°, the absolute maximum value of the depth of the groove in the magnetic domain control treatment line was non-uniform for each measurement point of the groove, and σ²(Dₘ) > 3.0 was further satisfied. The evaluation results of iron loss and noise of Example No. B3 were further superior to those of Example Nos. B1 and B2.

In Example No. B4, in addition to satisfying |β_{All}|-|β_{Dr}| ≥ 0.1°, the absolute maximum value of the depth of the groove in the magnetic domain control treatment line was non-uniform for each measurement point of the groove, and D_{m(β < βDr)} > D_{m(β≥ βDr)} was further satisfied. The evaluation results of iron loss and noise of Example No. B4 were further superior to those of Example Nos. B1 and B2.

In Example No. B5, in addition to satisfying |β_{All}|-|β_{Dr}| ≥ 0.1°, the absolute maximum value of the depth of the groove in the magnetic domain control treatment line was non-uniform for each measurement point of the groove, and σ²(Dₘ) > 3.0 and D_{m(β< βDr)} > D_{m(β≥ βDr)} were further satisfied. The evaluation results of iron loss and noise of Example No. B5 were the best among those of Example Nos. B1 to B5.

In Example No. B6, in addition to satisfying |β_{All}|-|β_{Dr}| ≥ 0.1°, the absolute maximum value of the depth of the groove in the magnetic domain control treatment line was non-uniform for each measurement point of the groove, and |β_{All}|-|β_{Dr}| > σ_{All}/2 was further satisfied. The evaluation results of iron loss and noise of Example No. B6 were further superior to those of Example Nos. B1 and B2.

In Example No. B7, in addition to satisfying |β_{All}|-|β_{Dr}| ≥ 0.1°, the absolute maximum value of the depth of the groove in the magnetic domain control treatment line was non-uniform for each measurement point of the groove, and |β_{All}|-|β_{Dr}| > σ_{All}/2 was satisfied in addition to satisfying σ²(Dₘ) > 3.0. The evaluation results of iron loss and noise of Example No. B7 were further superior to those of Example Nos. B1, B2, and B6.

In Example No. B8, in addition to satisfying |β_{All}|-|β_{Dr}| ≥ 0.1°, the absolute maximum value of the depth of the groove in the magnetic domain control treatment line was non-uniform for each measurement point of the groove, and |β_{All}|-|β_{Dr}| > σ_{All}/2 was satisfied in addition to satisfying D_{m(β < βDr)} > D_{m(β ≥ βDr)}. The evaluation results of iron loss and noise of Example No. B8 were further superior to those of Example Nos. B1, B2, and B6.

In Example No. B9 in addition to satisfying |β_{All}|-|β_{Dr}| ≥ 0.1°, the absolute maximum value of the depth of the groove in the magnetic domain control treatment line was non-uniform for each measurement point of the groove, and |β_{All}|-|β_{Dr}| > σ_{All}/2 was satisfied in addition to satisfying σ²(Dₘ) > 3.0 and D_{m(β< βDr)} > D_{m(β≥ βDr)}. At least one of the evaluation results of the iron loss and the noise of Example No. B9 was more excellent than B1 to B5 and B6 to B8.

In Example No. B10 in addition to satisfying |β_{All}|-|β_{Dr}| ≥ 0.1°, the absolute maximum value of the depth of the groove in the magnetic domain control treatment line was non-uniform for each measurement point of the groove, and σ_{Dr} < σ_{All} was satisfied. The evaluation results of iron loss and noise of Example No. B10 were further superior to those of Example Nos. B1 and B2.

In Example No. B11 in addition to satisfying |β_{All}|-|β_{Dr}| ≥ 0.1°, the absolute maximum value of the depth of the groove in the magnetic domain control treatment line was non-uniform for each measurement point of the groove, and σ_{Dr} < σ_{All} was satisfied in addition to satisfying σ²(Dₘ) > 3.0. At least one of the evaluation results of the iron loss and the noise of Example No. B7 was more excellent than those of Example Nos. B1, B2, and B10.

In Example No. B12 in addition to satisfying |β_{All}|-|β_{Dr}| ≥ 0.1°, the absolute maximum value of the depth of the groove in the magnetic domain control treatment line was non-uniform for each measurement point of the groove, and σ_{Dr} < σ_{All} was satisfied in addition to satisfying D_{m(β < βDr)} > D_{m(β ≥ βDr)}. The evaluation results of iron loss and noise of Example No. B12 were further superior to those of Example Nos. B1, B2, and B10.

In Example No. B13, in addition to satisfying |β_{All}|-|β_{Dr}| ≥ 0.1°, the absolute maximum value of the depth of the groove in the magnetic domain control treatment line was non-uniform for each measurement point of the groove, and σ_{Dr} < σ_{All} was satisfied in addition to satisfying σ²(Dₘ) > 3.0 and D_{m(β < βDr)} > D_{m(β ≥ βDr)}. At least one of the evaluation results of the iron loss and the noise of Example No. B13 was more excellent than B1 to B5 and B10 to B12.

In Example No. B14, in addition to satisfying |β_{All}|-|β_{Dr}| ≥ 0.1°, the absolute maximum value of the depth of the groove in the magnetic domain control treatment line was non-uniform for each measurement point of the groove, and |β_{All}|-|β_{Dr}| > σ_{All}/2 and σ_{Dr} < σ_{All} were satisfied in addition to satisfying σ²(Dₘ) > 3.0 and D_{m(β < βDr)} > D_{m(β ≥ βDr)}. The evaluation results of iron loss and noise of Example No. B14 were the best among B1 to B14.

### REFERENCE SIGNS LIST

1 Grain-oriented electrical steel sheet
11 Magnetic domain control treatment line
12A Region where the β angle is small
12B Region with large β angle
RD Rolling direction
TD Transverse direction
ND Rolled surface normal direction
VL1 Imaginary line parallel to TD for |β_{All}| calculation
VL2 Imaginary line parallel to RD for |β_{All}| calculation
VL3 Imaginary line parallel to TD for |β_{Dr}| calculation
VP1 Intersection point of imaginary line VL1 and imaginary line VL2
VP2 Magnetic domain control point
2 Original sheet
21 Magnetic domain control treatment region
22 Non-magnetic domain control treatment region
30 Image acquisition device
31 Light source unit
33 MO sensor
35 Image sensor
37 Signal processing unit
40 Analysis device
41 Calculation unit
43 Memory
45 Display unit
47 Input unit
49 Communication I/F
500 Laser irradiation device
501 Polygon mirror
503 light source device
505 Collimator
507 Condensing lens
509 Motor
511 Sensor
513 Control unit
515 Sheet passing device

## Claims

1. A grain-oriented electrical steel sheet having a magnetic domain control treatment line on a surface thereof, wherein
|β_{All}|-|β_{Dr}| ≥ 0.1° is satisfied,
|β_{All}| is an average value of absolute values of β angles over an entire surface of the grain-oriented electrical steel sheet, and
|β_{Dr}| is an average value of absolute values of β angles at magnetic domain control points that are intersection points of a plurality of the imaginary lines set at intervals of 2 mm in parallel along a rolling direction of the grain-oriented electrical steel sheet and the magnetic domain control treatment line.

2. The grain-oriented electrical steel sheet according to claim 1, wherein |β_{All}|-|β_{Dr}| ≥ 0.2° is satisfied.

3. The grain-oriented electrical steel sheet according to claim 1, wherein |β_{All}|-|β_{Dr}| ≥ 0.5° is satisfied.

4. The grain-oriented electrical steel sheet according to claim 1, wherein |β_{All}|-|β_{Dr}| ≥ 1.0° is satisfied.

5. The grain-oriented electrical steel sheet according to any one of claims 1 to 4, wherein
|β_{All}|-|β_{Dr}| > σ_{All}/2 is satisfied,
σ_{All} is a standard deviation of the absolute value of the β angle over the entire surface of the grain-oriented electrical steel sheet.

6. The grain-oriented electrical steel sheet according to any one of claims 1 to 4, wherein
σ_{Dr} < σ_{All} is satisfied,
σ_{All} is a standard deviation of the absolute value of the β angle over the entire surface of the grain-oriented electrical steel sheet, and
σ_{Dr} is a standard deviation of the absolute value of the β angle at the magnetic domain control point.

7. The grain-oriented electrical steel sheet according to any one of claims 1 to 4, wherein the magnetic domain control treatment line is a thermal strain.

8. The grain-oriented electrical steel sheet according to any one of claims 1 to 4, wherein the magnetic domain control treatment line is a groove.

9. The grain-oriented electrical steel sheet according to claim 7, wherein an absolute maximum value of tensile strength introduced into the thermal strain in the magnetic domain control treatment line is non-uniform at each measurement point of the tensile strength.

10. The grain-oriented electrical steel sheet according to claim 9, wherein
σ²(TSₘ) > 5.0 is satisfied,
TSₘ is the tensile strength in a unit of MPa introduced into the thermal strain measured at each of a plurality of the magnetic domain control points, and
σ²(TSₘ) is a variance of TSₘ.

11. The grain-oriented electrical steel sheet according to claim 9 or 10, wherein
TS_{m(β < βDr)} > TS_{m(β ≥ βDr)} is satisfied,
TS_{m(β < βDr)} is an arithmetical mean value of the absolute maximum value of the tensile strength in a unit of MPa introduced in the thermal strain measured at each of the magnetic domain treatment points having a β angle of less than β_{Dr} among the magnetic domain treatment points, and
TS_{m(β ≥ βDr)} is an arithmetical mean value of the absolute maximum value of the tensile strength in a unit of MPa introduced into the thermal strain measured at each of the magnetic domain treatment points having the β angle of β_{Dr} or more.

12. The grain-grain-oriented electrical steel sheet according to claim 8, wherein an absolute maximum value of a depth of the groove in the magnetic domain control treatment line is non-uniform at each measurement point of the groove.

13. The grain-oriented electrical steel sheet according to claim 12, wherein
σ²(Dₘ) > 3.0 is satisfied,
Dₘ is an absolute maximum value of a depth of the groove in a unit of µm at the magnetic domain control point, and
σ²(Dₘ) is the variance of Dₘ.

14. The grain-oriented electrical steel sheet according to claim 12 or 13, wherein
D_{m(β < βDr)} > D_{m(β ≥ βDr)} is satisfied,
D_{m(β < βDr)} is an arithmetical mean value of absolute maximum values of the depths of the grooves in a unit µm measured at each of the magnetic domain control points having a β angle of less than β_{Dr} among the magnetic domain control points, and
D_{m(β ≥ βDr)} is an arithmetical mean value of absolute maximum values of the depths of the grooves in a unit µm measured at each of the magnetic domain control points having the β angle of β_{Dr} or more.

15. Method for manufacturing a grain-oriented electrical steel sheet comprising:
a step of acquiring a magnetic domain image of an original sheet of a grain-oriented electrical steel sheet;
a step of determining a magnetic domain control treatment region based on a distribution of spacing of magnetic domain walls in the magnetic domain image; and
a step of applying a magnetic domain control treatment to the magnetic domain control treatment region determined based on a distribution of a spacing of magnetic domain walls; wherein
in the grain-oriented electrical steel sheet to which the magnetic domain control treatment is applied, |β_{All}|-|β_{Dr}| ≥ 0.1° is set, and
|β_{All}| is an average value of absolute values of β angles over an entire surface of the grain-oriented electrical steel sheet to which the magnetic domain control treatment is applied, and
|β_{Dr}| is an average value of absolute values of β angles at magnetic domain control points that are intersection points of a plurality of imaginary lines set at intervals of 2 mm in parallel along a rolling direction of the grain-oriented electrical steel sheet to which the magnetic domain control treatment is applied and a magnetic domain control treatment line formed by the magnetic domain control treatment.

16. The method for manufacturing a grain-oriented electrical steel sheet according to claim 15, wherein a region where the spacing of magnetic domain walls is a predetermined value or more is set as the magnetic domain control treatment region.

17. The method for manufacturing a grain-oriented electrical steel sheet according to claim 15 or 16, wherein a distribution of the spacing of magnetic domain walls is derived from the magnetic domain image using a two-dimensional Fourier transform.

18. The method for manufacturing a grain-oriented electrical steel sheet according to claim 15 or 16, wherein the magnetic domain control treatment is applied by irradiation with a laser or an electron beam.

19. The method for manufacturing a grain-oriented electrical steel sheet according to claim 15, wherein a magnetic domain control strength is made non-uniform in the step of applying the magnetic domain control treatment to the magnetic domain control treatment region.
